



US011796930B2

(12) **United States Patent**  
**Watanabe et al.**

(10) **Patent No.:** **US 11,796,930 B2**  
(b4) **Date of Patent:** **Oct. 24, 2023**

(54) **MAGNETIC TONER**(71) Applicant: **CANON KABUSHIKI KAISHA**,  
Tokyo (JP)(72) Inventors: **Shuntaro Watanabe**, Kanagawa (JP);  
**Hiroki Akiyama**, Shizuoka (JP); **Hiroki**  
**Kagawa**, Shizuoka (JP)(73) Assignee: **CANON KABUSHIKI KAISHA**,  
Tokyo (JP)(\*) Notice: Subject to any disclaimer, the term of this  
patent is extended or adjusted under 35  
U.S.C. 154(b) by 192 days.(21) Appl. No.: **17/168,523**(22) Filed: **Feb. 5, 2021**(65) **Prior Publication Data**

US 2021/0255557 A1 Aug. 19, 2021

(30) **Foreign Application Priority Data**

Feb. 14, 2020 (JP) ..... 2020-023197

(51) **Int. Cl.****G03G 9/083** (2006.01)  
**G03G 9/087** (2006.01)(52) **U.S. Cl.**CPC ..... **G03G 9/0837** (2013.01); **G03G 9/0832**  
(2013.01); **G03G 9/0836** (2013.01); **G03G**  
**9/08755** (2013.01)(58) **Field of Classification Search**CPC .. G03G 9/0837; G03G 9/0832; G03G 9/0836;  
G03G 9/08755

See application file for complete search history.

(56) **References Cited**

## U.S. PATENT DOCUMENTS

|                |         |                  |                          |
|----------------|---------|------------------|--------------------------|
| 7,014,969 B2   | 3/2006  | Yachi et al.     |                          |
| 8,603,712 B2   | 12/2013 | Aoki et al.      |                          |
| 8,741,519 B2   | 6/2014  | Watanabe et al.  |                          |
| 8,785,101 B2   | 7/2014  | Kaya et al.      |                          |
| 8,846,284 B2   | 9/2014  | Kinumatsu et al. |                          |
| 9,029,055 B2 * | 5/2015  | Aoki             | G03G 9/0833<br>430/106.1 |
| 9,201,323 B2   | 12/2015 | Nishikawa et al. |                          |
| 9,250,548 B2   | 2/2016  | Nomura et al.    |                          |
| 9,261,804 B2   | 2/2016  | Yamazaki et al.  |                          |
| 9,309,349 B2   | 4/2016  | Watanabe et al.  |                          |
| 9,341,970 B2   | 5/2016  | Yoshida et al.   |                          |
| 9,429,860 B2   | 8/2016  | Kinumatsu et al. |                          |
| 9,470,993 B2   | 10/2016 | Nishikawa et al. |                          |
| 9,606,462 B2   | 3/2017  | Nomura et al.    |                          |
| 9,625,844 B2   | 4/2017  | Kaya et al.      |                          |
| 9,658,554 B2   | 5/2017  | Kinumatsu et al. |                          |
| 9,798,256 B2   | 10/2017 | Kosaki et al.    |                          |
| 9,798,262 B2   | 10/2017 | Toyoizumi et al. |                          |

|                   |         |                                        |
|-------------------|---------|----------------------------------------|
| 9,811,016 B2      | 11/2017 | Aoki et al.                            |
| 9,823,595 B2      | 11/2017 | Toyoizumi et al.                       |
| 9,829,818 B2      | 11/2017 | Yoshida et al.                         |
| 9,857,713 B2      | 1/2018  | Kosaki et al.                          |
| 9,869,943 B2      | 1/2018  | Aoki et al.                            |
| 10,101,683 B2     | 10/2018 | Nishikawa et al.                       |
| 10,409,180 B2     | 9/2019  | Koji et al.                            |
| 10,545,420 B2 *   | 1/2020  | Kinumatsu ..... G03G 9/08764           |
| 10,747,134 B2     | 8/2020  | Watanabe et al.                        |
| 10,768,540 B2     | 9/2020  | Watanabe et al.                        |
| 2010/0035171 A1   | 2/2010  | Watanabe et al.                        |
| 2014/0099579 A1 * | 4/2014  | Takagi ..... G03G 9/1137<br>430/124.1  |
| 2014/0348550 A1 * | 11/2014 | Nagayama ..... G03G 15/0877<br>399/262 |
| 2016/0161874 A1   | 6/2016  | Yamazaki et al.                        |
| 2017/0336726 A1 * | 11/2017 | Hasegawa ..... G03G 9/0926             |
| 2018/0129146 A1 * | 5/2018  | Kawamura ..... G03G 9/0825             |
| 2019/0384192 A1   | 12/2019 | Kagawa et al.                          |
| 2019/0384195 A1   | 12/2019 | Saeki et al.                           |
| 2020/0081361 A1   | 3/2020  | Yoshida et al.                         |
| 2020/0285164 A1   | 9/2020  | Akiyama et al.                         |
| 2021/0055667 A1   | 2/2021  | Watanabe et al.                        |
| 2021/0080846 A1   | 3/2021  | Mizuguchi et al.                       |

## FOREIGN PATENT DOCUMENTS

|    |              |         |
|----|--------------|---------|
| JP | 2005338538 A | 12/2005 |
| JP | 2013137420 A | 7/2013  |
| JP | 2019003129 A | 1/2019  |
| JP | 2019015957 A | 1/2019  |

## OTHER PUBLICATIONS

U.S. Appl. No. 17/197,102, Yuujiro Nagashima, filed Mar. 10, 2021.

\* cited by examiner

Primary Examiner — Peter L Vajda

Assistant Examiner — Boone Alexander Evans

(74) Attorney, Agent, or Firm — VENABLE LLP

(57) **ABSTRACT**

A magnetic toner comprising a magnetic toner particle including a binder resin, a magnetic body and a crystalline polyester, wherein in cross-sectional observation of the magnetic toner particle using a transmission electron microscope, a variation coefficient CV3 of an occupied area ratio of the magnetic body when a cross section of the magnetic toner particle is divided by a square grid having a side of 0.8  $\mu\text{m}$  is from 40.0% to 80.0%, and assuming that a storage elastic modulus at 40° C. is taken as  $E'(40)$  [Pa] and a storage elastic modulus at 85° C. is taken as  $E'(85)$  [Pa], the storage elastic moduli being obtained in a powder dynamic viscoelasticity measurement of the magnetic toner, the following formulas (1) and (2) are satisfied.

$$E'(85) \leq 2.0 \times 10^9 \quad (1)$$

$$[E'(40) - E'(85)] \times 100 / E'(40) \geq 70 \quad (2)$$

7 Claims, No Drawings

## 1

## MAGNETIC TONER

## BACKGROUND OF THE INVENTION

## Field of the Invention

The present invention relates to a magnetic toner for use in a recording method using electrophotography, electrostatic recording, or toner jet recording.

## Description of the Related Art

In recent years, a demand has been created for means for outputting images in a wide range of fields from offices to homes and in various environments, and high image quality is required under all of these circumstances. Meanwhile, downsizing and energy saving are also required for the image output apparatus itself.

In order to save energy, it is important that the toner be sufficiently fixed at a low temperature.

The usage of a crystalline polyester that becomes rapidly compatible with the binder resin of a toner and promotes the melt deformation of the toner particle in the toner, and the control of viscoelastic properties of the toner have been widely studied as means for improving the fixability. A crystalline polyester producing a high effect on low-temperature fixability has the property of easily becoming compatible with the binder resin in the vicinity of the melting point thereof, and the toner including the crystalline polyester is easily melted and deformed rapidly at the time of fixing. Therefore, the low-temperature fixability of the toner is improved by using the crystalline polyester. Japanese Patent Application Publication No. 2013-137420 proposes a toner including a crystalline polyester.

Meanwhile, miniaturization of the cartridge accommodating the developer is an effective means for reducing the size of the image output device. Among the development methods, a one-component development method is preferable to a two-component development method using a carrier, and makes it possible to reduce the weight of the cartridge. Further, in order to reduce a mechanical load on the toner, a non-contact developing method is preferable to a contact developing method in which a photosensitive member and the toner bearing member are in contact with each other. Therefore, the one-component non-contact developing method is an effective means for satisfying miniaturization and high image quality.

In the one-component non-contact developing method, a toner bearing member and an electrostatic latent image bearing member are arranged in a non-contact manner. That is, the toner including magnetic bodies is conveyed by rotating the bearing member incorporating a magnet. Since the resistance value of the magnetic bodies is lower than that of the binder resin, the charging performance of the toner changes depending on the presence state of the magnetic bodies inside the toner.

Japanese Patent Application Publication No. 2005-338538 proposes a toner obtained by a dry method in which magnetic bodies are uniformly dispersed inside the toner by controlling the acid value and hydroxy value of a binder resin and the oil absorption amount and true density of the magnetic bodies.

## SUMMARY OF THE INVENTION

However, it has been found that in the toner of Japanese Patent Application Publication No. 2005-338538, the

## 2

improvement of the dispersibility of the magnetic bodies leads to the exposure of the magnetic bodies on the toner surface, and it is difficult to maintain the charge quantity of the toner in a high-temperature and high-humidity environment.

A core-shell type toner in which a surface layer is provided on the toner particle surface in order to suppress exposure of magnetic bodies on the toner surface can be considered.

10 Japanese Patent Application Publication No. 2019-3129 proposes a core-shell type toner including magnetic bodies that is obtained by a suspension polymerization method. However, it has been found that the magnetic bodies are unevenly distributed to the toner surface, the surface adhesion between the toner particles becomes insufficient when the toner is fixed at a low temperature, and the wear resistance of the image is weakened.

Further, Japanese Patent Application Publication No. 2019-15957 proposes a magnetic toner in which magnetic bodies are dispersed by using an emulsion aggregation method in order to maintain appropriate dispersibility while suppressing exposure of the magnetic bodies on the toner surface.

However, it has been found that it is necessary to include 25 a large amount of a crystalline polyester having a sharp melt property in a binder resin in order to improve the low-temperature fixability so as to meet the above-mentioned request for energy saving.

In the toners disclosed in the above document, when a 30 large amount of a crystalline resin is added in order to improve the low-temperature fixability, the dispersibility of the magnetic bodies is lowered, and the magnetic bodies aggregate inside the toner thereby reducing the tinting strength. It was also found that the affinity between the 35 low-polarity crystalline resin and the magnetic bodies is low, and thus the possibility of occurrence of exposure of the magnetic bodies on the toner surface and a charge leak are high. As a result, it was found that toner deterioration is likely to occur in harsh environments such as high-temperature 40 and high-humidity environment and low-temperature and low-humidity environment.

Depending on the combination of the composition of the 45 crystalline polyester added in a large amount, the composition of the binder resin, and surface properties and surface 50 polarity of the magnetic bodies, the dispersed state of the magnetic bodies inside the toner can become non-uniform and there can be a spread in the amount of magnetic bodies contained in the toner particles. Such a presence state of the 55 magnetic bodies degrades the charging performance of the toner, lowers the developing performance, and degrades the uniformity of image density. Further, the above-described means were found to be insufficient to suppress melting unevenness and electrostatic offset caused by the magnetic bodies when the toner is fixed in a low-temperature and low-humidity environment.

The present disclosure provides a magnetic toner that is 60 resistant to environmental changes, has excellent low-temperature fixability, and makes it possible to suppress toner melting unevenness and electrostatic offset even in a harsh environment.

The inventors of the present invention have found that the above problems can be solved by controlling the dispersed state of magnetic bodies in the magnetic toner and the storage elastic modulus of the magnetic toner.

65 The present disclosure relates to a magnetic toner comprising a magnetic toner particle comprising a binder resin, a magnetic body and a crystalline polyester, wherein

in cross-sectional observation of the magnetic toner particle using a transmission electron microscope,

a variation coefficient CV3 of an occupied area ratio of the magnetic body when a cross section of the magnetic toner particle is divided by a square grid having a side of 0.8  $\mu\text{m}$  is 40.0 to 80.0%, and

assuming that a storage elastic modulus at 40° C. is defined as  $E'(40)$  [Pa] and a storage elastic modulus at 85° C. is defined as  $E'(85)$  [Pa], the storage elastic moduli being obtained in a powder dynamic viscoelasticity measurement of the magnetic toner, the following formulas (1) and (2) are satisfied.

$$E'(85) \leq 2.0 \times 10^9 \quad (1)$$

$$[E'(40) - E'(85)] \times 100/E'(40) \geq 70 \quad (2)$$

The present disclosure can provide a magnetic toner that is resistant to environmental changes, has excellent low-temperature fixability, and makes it possible to suppress toner melting unevenness and electrostatic offset even in a harsh environment.

Further features of the present invention will become apparent from the following description of exemplary embodiments.

#### DESCRIPTION OF THE EMBODIMENTS

In the present invention, the descriptions of "from XX to YY" or "XX to YY" representing a numerical range mean a numerical range including the lower limit and the upper limit which are endpoints, unless otherwise noted.

Further, a monomer unit means the reacted form of a monomer substance in a polymer.

Where a numerical range is described step by step, the upper and lower limits of each numerical range can be arbitrarily combined.

Hereinafter, the magnetic toner will be described in greater detail, but the present invention is not limited thereto.

The present disclosure relates to a magnetic toner comprising a magnetic toner particle that comprising a binder resin, a magnetic body and a crystalline polyester, wherein in cross-sectional observation of the magnetic toner particle using a transmission electron microscope,

a variation coefficient CV3 of an occupied area ratio of the magnetic body when a cross section of the magnetic toner particle is divided by a square grid having a side of 0.8  $\mu\text{m}$  is 40.0 to 80.0%, and

assuming that a storage elastic modulus at 40° C. is defined as  $E'(40)$  [Pa] and a storage elastic modulus at 85° C. is defined as  $E'(85)$  [Pa], the storage elastic moduli being obtained in a powder dynamic viscoelasticity measurement of the magnetic toner, the following formulas (1) and (2) are satisfied.

$$E'(85) \leq 2.0 \times 10^9 \quad (1)$$

$$[E'(40) - E'(85)] \times 100/E'(40) \geq 70 \quad (2)$$

In the magnetic toner, the dispersion state of magnetic bodies in a magnetic toner particle (hereinafter, also simply referred to as toner particle) is controlled to control the storage elastic moduli of the magnetic toner.

The inventors of the present invention have found a method for solving the problems of improving the low-temperature fixability and suppressing the electrostatic offset by setting the storage elastic modulus of the magnetic toner within a specific range.

However, regarding the durability, a problem was associated with developing performance during durability.

The inventors of the present invention thought that the sharp melt property in a toner to which a large amount of crystalline resin is added will be improved by including a segment that does not include a magnetic body so that the crystalline resin could easily form a domain.

Thus, it was thought that the location where the binder resin is unevenly distributed in the magnetic toner particle, that is, the presence of a domain of the binder resin in the toner particle, is an effective solution for the problem of sharp melting property of the toner particle.

The inventors of the present invention have found a means capable of forming a state in which magnetic bodies are aggregated to some extent in each toner particle. As a result, a toner which is excellent in low-temperature fixability and storage stability was obtained, and the present invention has been accomplished.

In the magnetic toner, in cross-sectional observation of the magnetic toner particle using a transmission electron microscope (TEM), a variation coefficient CV3 of an occupied area ratio of magnetic bodies when a cross section of the magnetic toner particle is divided by a square grid having a side of 0.8  $\mu\text{m}$  is from 40.0% to 80.0%. The CV3 is preferably from 45.0% to 70.0%.

The fact that the CV3 is in the above range means that the magnetic bodies are unevenly localized in the magnetic toner particle. That is, by unevenly distributing the magnetic bodies in the magnetic toner particle, it is possible to appropriately provide a portion where the magnetic body is not present (that is, the domain portion of the binder resin), and crystallize the crystalline polyester in this portion.

As a result, a sharp melt property of the toner particles is promoted, and the adhesion of the toner to the medium such as paper when a large number of images are outputted can be improved under the condition of a high process speed.

Further, since the magnetic bodies are not excessively exposed on the toner particle surface, a satisfactory image with a small electrostatic offset can be obtained, leak of charge of the toner particle can be suppressed and developing performance during durability is improved. Further, by dispersing the magnetic bodies in the toner particles in an appropriately aggregated state, it becomes possible to improve the storage elastic modulus at low temperature and to increase the value of  $E'(40)$  [Pa].

When the CV3 is less than 40.0%, the difference in the occupied area ratio of the magnetic bodies is small between the grids that divide the cross section of the magnetic toner particle. That is, it means that the domain portions of the binder resin including the crystallized crystalline polyester are not present, or the amount of present domain portions of the binder resin including the crystallized crystalline polyester is small.

In this case, most of the crystalline polyester forms a fine network structure, and the connections between the crystalline polyester portions become thin. As a result, the sharp melt property of the toner particles is inhibited, and the low-temperature fixability is lowered. In addition, the magnetic bodies become overdispersed, and it becomes difficult to maintain the elasticity of the entire toner at the time of melting, so that the fixing separability is lowered.

Meanwhile, when the CV3 exceeds 80.0%, the magnetic bodies are excessively localized in the toner. In this case, when the magnetic bodies aggregate with each other and the toner gets wet and spreads at the time of fixing, the tinting strength decreases due to the decrease in the shielding power, and the image density in the initial period of image

output decreases. In addition, since the magnetic bodies are likely to be present near the toner surface, the magnetic bodies tend to migrate from the toner surface, and the image density difference between before and after durable use becomes large (image density uniformity decreases).

Controlling the hydrophilicity/hydrophobicity, BET specific surface area and oil absorption amount on the surface of the magnetic bodies, and controlling the degree of aggregation of the magnetic bodies at the time of production of toner particles, and the like can be mentioned as methods for adjusting the CV3 in the above range.

For example, in the case of using an emulsion aggregation method, a method of aggregating the magnetic bodies in advance and introducing the aggregate into the toner particle, a method of adding a chelating agent and/or adjusting the pH in the coalescence step to adjust the degree of aggregation of the magnetic bodies, and the like can be used.

Further, in cross-sectional observation of a magnetic toner particle using a transmission electron microscope (TEM), the average value of the occupied area ratio of the magnetic body when a cross section of the magnetic toner particle is divided by a square grid having aside of  $0.8 \mu\text{m}$  is from 10.0% to 40.0%, and more preferably from 15.0% to 30.0%.

When the average value of the occupied area ratio of the magnetic body is in the above range, the dispersed state of the magnetic bodies in the toner particle becomes appropriate, and it is possible to suppress the decrease in tinting strength due to the excessive aggregation state.

Further, the amount of the present binder resin domains is appropriate, and the toner particle is less likely to be cracked. As a result, the electrostatic offset and the decrease in fixing separability hardly occur, and a satisfactory image can be obtained. In addition, controlling the hydrophilicity/hydrophobicity of the surface of the magnetic body, controlling the degree of aggregation of the magnetic bodies at the time of production of toner particles, and the like can be mentioned as methods for controlling the average value of the occupied area ratio of the magnetic body in the above range.

Where the storage elastic modulus at  $40^\circ\text{C}$ . is defined as  $E'(40)$  [Pa] and the storage elastic modulus at  $85^\circ\text{C}$ . is defined as  $E'(85)$  [Pa], the storage elastic moduli being obtained in a powder dynamic viscoelasticity measurement of the magnetic toner, the following formulas (1) and (2) are satisfied:

$$E'(85) \leq 2.0 \times 10^9 \quad (1)$$

$$[E'(40) - E'(85)] \times 100 / E'(40) \geq 70 \quad (2)$$

When  $E'(85)$  satisfies the above formula (1), the elasticity of the toner at the time of fixing becomes appropriate, and the adhesion to paper becomes strong, so that the low-temperature fixability is improved, durability of the image against rubbing is increased, electrostatic offset in a low-temperature environment can be suppressed, and a satisfactory image can be obtained.

When  $E'(85)$  exceeds  $2.0 \times 10^9$ , the elasticity is too high, and the adhesion to paper is lowered, so that the low-temperature fixability is lowered and the electrostatic offset tends to occur.

$E'(85)$  can be controlled by the storage modulus of the binder resin and the addition amount of the crystalline polyester. The storage elastic modulus of the binder resin can be controlled by appropriately adjusting the types and molecular weights of constituent monomers.

Further,  $E'(85)$  is preferably  $1.0 \times 10^9$  or less, and more preferably  $0.7 \times 10^9$  or less.

The lower limit of  $E'(85)$  is not particularly limited, but is preferably  $0.1 \times 10^9$  or more, and more preferably  $0.2 \times 10^9$  or more.

The fact that  $E'(40)$  and  $E'(85)$  satisfy the formula (2) indicates that the magnetic toner can undergo a rapid elastic change at  $40^\circ\text{C}$ . to  $85^\circ\text{C}$ . As a result, even in the fixing step with a high process speed, the toner is sufficiently sharp-melted, the adhesion of the toner to the paper is improved, and low-temperature fixing becomes possible.

When  $[E'(40) - E'(85)] \times 100 / E'(40)$  is less than 70, elastic change does not occur at  $40^\circ\text{C}$ . to  $85^\circ\text{C}$ ., and the sharp melt property of the toner becomes insufficient. Therefore, since the toner does not melt to a predetermined elasticity in a short time, the low-temperature fixability is lowered.

$[E'(40) - E'(85)] \times 100 / E'(40)$  is preferably 72 or more. Meanwhile, the upper limit is not particularly limited, but is preferably 90 or less, more preferably 85 or less, and still more preferably 80 or less.

$E'(40)$  and  $E'(85)$  can be controlled by the storage modulus of the binder resin and the addition amount of the crystalline polyester. The storage elastic modulus of the binder resin can be controlled by appropriately adjusting the types and molecular weights of constituent monomers.

The magnetic toner particle preferably further comprises wax (release agent).

Assuming that the peak temperature of the maximum endothermic peak at the time of the first temperature rise that is assigned to the crystalline polyester in the differential scanning calorimetry of the magnetic toner is defined as  $T_{m(1)}$   $^\circ\text{C}$ ., the endothermic quantity of the maximum endothermic peak is defined as  $H(1)$  J/g, and the peak temperature of the maximum endothermic peak assigned to wax is taken as  $T_{m(2)}$   $^\circ\text{C}$ ., it is preferable that the following formulas (3) to (5) are satisfied.

$$5.0 \leq T_{m(2)} - T_{m(1)} \leq 35.0 \quad (3)$$

$$55.0 \leq T_{m(2)} \leq 100.0 \quad (4)$$

$$H(1) \geq 10.0 \quad (5)$$

Where  $T_{m(2)} - T_{m(1)}$  is  $5.0^\circ\text{C}$ . or higher, the crystalline polyester and the wax are unlikely to be compatible with each other, the crystallinity of the crystalline polyester is satisfactorily maintained, the sharp melt property of the toner is improved, and the low-temperature fixability is improved.

Where  $T_{m(2)} - T_{m(1)}$  is  $35.0^\circ\text{C}$ . or lower, the wax easily bleeds out when the binder resin is melted at a high temperature, so that the fixing releasability is improved and paper curling can be suppressed.

$T_{m(2)} - T_{m(1)}$  is more preferably from  $10.0^\circ\text{C}$ . to  $25.0^\circ\text{C}$ .

The melting point  $T_{m(2)}$  of the wax is preferably from  $55.0^\circ\text{C}$ . to  $100.0^\circ\text{C}$ . Where  $T_{m(2)}$  is  $55^\circ\text{C}$ . or higher, the wax is less likely to be exposed on the toner particle surface, and the heat-resistant storage stability is improved. Where  $T_{m(2)}$  is  $100.0^\circ\text{C}$ . or lower, the wax bleeds out when the binder resin is melted, and the low-temperature fixability is improved.

$T_{m(2)}$  is more preferably from  $60.0^\circ\text{C}$ . to  $90.0^\circ\text{C}$ .

Where the endothermic quantity  $H(1)$  is  $10.0 \text{ J/g}$  or more, the domains of the crystalline polyester in the binder resin become appropriately large, so that the binder resin is likely to be plasticized by melting the crystalline polyester during low-temperature fixing, thereby improving low-temperature fixability.

H(1) is more preferably 12.0 J/g or more. The upper limit is not particularly limited, but is preferably 30.0 J/g or less, and more preferably 27.0 J/g or less.

The toner particle includes crystalline polyester. The crystalline polyester is preferably a condensation polymerization product of a monomer including an aliphatic diol and/or an aliphatic dicarboxylic acid. The crystalline resin, as referred to herein, means a resin which shows a clear melting point by the measurement using a differential scanning calorimeter (DSC).

The crystalline polyester preferably includes a monomer unit derived from an aliphatic diol having 2 to 12 carbon atoms, and/or a monomer unit derived from an aliphatic dicarboxylic acid having 2 to 12 carbon atoms.

Examples of the aliphatic diol having from 2 to 12 carbon atoms include the following compounds.

1,2-Ethanediol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-undecanediol, and 1,12-dodecanediol.

In addition, an aliphatic diol having a double bond can also be used. The aliphatic diol having a double bond can be exemplified by the following compounds.

2-Butene-1,4-diol, 3-hexene-1,6-diol and 4-octene-1,8-diol.

The aliphatic dicarboxylic acid having from 2 to 12 carbon atoms can be exemplified by the following compounds.

Oxalic acid, malonic acid, succinic acid, glutaric acid, adipic acid, pimelic acid, suberic acid, azelaic acid, sebacic acid, 1,9-nonanedicarboxylic acid, 1,10-decanedicarboxylic acid, 1,11-undecanedicarboxylic acid, 1,12-dodecanedicarboxylic acid. Lower alkyl esters and acid anhydrides of these aliphatic dicarboxylic acids can also be used.

Among these, sebacic acid, adipic acid and 1,10-decanedicarboxylic acid and lower alkyl esters and acid anhydrides thereof are preferred. These may be used singly or in combination of two or more thereof.

In addition, an aromatic carboxylic acid can also be used. The aromatic dicarboxylic acid can be exemplified by the following compounds. Terephthalic acid, isophthalic acid, 2,6-naphthalenedicarboxylic acid and 4,4'-biphenyldicarboxylic acid. Among these, terephthalic acid is preferable from the standpoint of easy availability and easy formation of a polymer having a low melting point.

Also, a dicarboxylic acid having a double bond can be used. The dicarboxylic acid having a double bond can be suitably used in order to suppress the hot offset at the time of fixing because such an acid makes it possible to crosslink the entire resin by using the double bond.

Such a dicarboxylic acid can be exemplified by fumaric acid, maleic acid, 3-hexenediolic acid and 3-octendienic acid. Also included are lower alkyl esters and acid anhydrides thereof. Among these, fumaric acid and maleic acid are more preferable.

A method for manufacturing a crystalline polyester is not particularly limited, and can be implemented by the general polymerization method of polyesters in which a dicarboxylic acid component and a diol component are reacted with each other. For example, direct polycondensation or transesterification can be used depending on the type of monomers.

The peak temperature of the maximum endothermic peak of the crystalline polyester measured using a differential scanning calorimeter (DSC) is preferably from 50.0° C. to 100.0° C., and more preferably, from the viewpoint of low-temperature fixability, from 60.0° C. to 90.0° C.

The weight average molecular weight Mw of the crystalline polyester is preferably from 5000 to 50000, and more preferably from 10000 to 45000.

The number average molecular weight Mn of the crystalline polyester is preferably from 1000 to 20000, and more preferably from 2000 to 15000.

The amount of the crystalline polyester is preferably 30.0% by mass or more based on the total amount of the binder resin and the crystalline polyester. More preferably, 10 the amount of the crystalline polyester is from 31.0% by mass to 60.0% by mass.

Where the amount of the crystalline polyester is 30.0% by mass or more, the crystalline polyester is contained in a preferred amount, so that the crystalline polyester plasticizes 15 the binder resin and the low-temperature fixability is improved.

Further, where the amount of the crystalline polyester is in the above range, the occupied area ratio of the magnetic body is unlikely to decrease, so that excessive aggregation 20 of the magnetic bodies can be suppressed, and a decrease in image density can be suppressed.

The magnetic toner particle may include a wax.

A well-known wax may be used. Specific examples of the wax are presented hereinbelow.

Petroleum waxes such as paraffin wax, microcrystalline wax, petrolactam and the like and derivatives thereof, montan wax and derivatives thereof, hydrocarbon waxes obtained by a Fischer-Tropsch method and derivatives thereof, polyolefin waxes represented by polyethylene and 30 polypropylene, and derivatives thereof, natural waxes such as carnauba wax, candelilla wax and derivatives thereof, ester waxes and the like.

Here, the derivatives include oxides, block copolymers with vinyl-based monomers, and graft modified products.

In addition, a monoester compound including one ester bond in a molecule and a polyfunctional ester compound such as a diester compound including two ester bonds in a molecule, a tetrafunctional ester compound including four ester bonds in a molecule, a hexafunctional ester compound 40 including six ester bonds in a molecule and the like can be used as the ester wax.

The ester wax preferably includes at least one compound selected from the group consisting of monoester compounds and diester compounds.

45 Specific examples of the monoester compounds include waxes mainly composed of a fatty acid ester, such as carnauba wax, montanic acid ester wax and the like; compounds obtained by partial or complete removal of the acid component from a fatty acid ester, such as a deacidified carnauba wax and the like, compounds obtained by hydrogenation of vegetable oils and fats, and the like, and methyl ester compounds having a hydroxy group; and saturated fatty acid monoesters such as stearyl stearate and behenyl behenate.

55 Further, specific examples of the diester compound include dibehenyl sebacate, nonanediol dibenenate, dibehenyl terephthalate, distearyl terephthalate and the like.

In addition, the wax can include well-known other waxes other than the abovementioned compounds. Further, one 60 type of wax may be used singly, or two or more types may be used in combination.

The amount of the wax is preferably from 1.0 part by mass to 30.0 parts by mass, and more preferably from 3.0 parts by mass to 25.0 parts by mass with respect to 100 parts by mass of the binder resin.

Examples of the magnetic body include iron oxides such as magnetite, maghemite, ferrite and the like; metals such as

iron, cobalt, nickel and the like, alloys of these metals with a metal such as aluminum, copper, magnesium, tin, zinc, beryllium, calcium, manganese, selenium, titanium, tungsten, vanadium and the like, and mixtures thereof.

The number average particle diameter of the primary particles of the magnetic bodies is preferably 0.50  $\mu\text{m}$  or less, and more preferably from 0.05  $\mu\text{m}$  to 0.30  $\mu\text{m}$ .

The number average particle diameter of the primary particles of the magnetic bodies present in the toner particle can be measured using a transmission electron microscope.

Specifically, after sufficiently dispersing toner particles to be observed in an epoxy resin, curing is performed in an atmosphere having a temperature of 40° C. for 2 days to obtain a cured product. The resulting cured product is sliced into a flaky sample by a microtome, an image at a magnification of 10,000 to 40,000 is captured in a transmission electron microscope (TEM), and the projected area of 100 primary particles of the magnetic bodies in the image is measured. Then, the equivalent diameter of the circle equal to the projected area is taken as the particle diameter of the primary particle of the magnetic body, and the average value of 100 particle diameters is taken as the number average particle diameter of the primary particles of the magnetic bodies.

The magnetic body has the oil absorption amount of preferably from 15.0 ml/100 g to 25.0 ml/100 g, and more preferably from 17.0 ml/100 g to 23.0 ml/100 g. Where the oil absorption amount is 15.0 ml/100 g or more, the magnetic bodies and the binding resin become more compatible with each other, and the magnetic bodies are less likely to aggregate, so that the coloring property of the toner is improved.

Where the oil absorption amount is 25.0 ml/100 g or less, the contact between the magnetic body and the ester bond of the crystalline polyester can be suppressed while improving the dispersibility of the magnetic bodies, and the chargeability of the toner is improved.

The magnetic body has the isoelectric point of preferably from pH 8.5 to pH 10.5, and more preferably from pH 8.5 to pH 10.0.

Where the isoelectric point is pH 8.5 or higher, in the emulsion aggregation method, the affinity between the magnetic body and the binding resin increases at the time of aggregation, and the magnetic bodies do not easily aggregate, so that the coloring property of the toner improves. Where the isoelectric point is pH 10.5 or less, the affinity between the magnetic body and water in the dispersion medium can be appropriately maintained in the emulsion aggregation method while improving the dispersibility of the magnetic bodies. Therefore, the magnetic bodies are less likely to be exposed on the toner particle surface, and moisture is less likely to be adsorbed on the toner surface in a high-temperature and high-humidity environment, so that the charge retention property is improved.

As a magnetic property of the magnetic body at 795.8 kA/m application, a coercive force (Hc) is preferably 1.6 kA/m to 12.0 kA/m. The magnetization strength (as) is preferably 50 Am<sup>2</sup>/kg to 200 Am<sup>2</sup>/kg, and more preferably 50 Am<sup>2</sup>/kg to 100 Am<sup>2</sup>/kg. Meanwhile, the residual magnetization (gr) is preferably 2 Am<sup>2</sup>/kg to 20 Am<sup>2</sup>/kg.

The amount of the magnetic bodies in the magnetic toner is preferably from 10.0% by mass to 50.0% by mass, and more preferably from 15.0% by mass to 45.0% by mass.

Where the amount of the magnetic bodies is 10.0% by mass or more, satisfactory magnetization of the toner particle can be maintained while improving the dispersibility of the magnetic bodies inside the toner particle, so that the

attraction force to the developer bearing member that maintains magnetism in the one-component non-contact development method can be satisfactorily controlled. Therefore, when an AC development bias is applied, fogging in the non-contact development method can be suppressed. In addition, the coloring property is also improved.

When the amount of the magnetic bodies is within the above range, the magnetic attraction with the magnet roll in the developing sleeve is appropriate.

The amount of the magnetic bodies in the magnetic toner can be measured using a thermal analyzer TGA Q5000IR manufactured by Perkin Elmer Co. The measurement method is as follows: the magnetic toner is heated from normal temperature to 900° C. at a temperature rise rate of 25° C./min in a nitrogen atmosphere, the mass lost at 100° C. to 750° C. is taken as the mass of the components other than the magnetic bodies in the magnetic toner, and the residual mass is taken as the mass of magnetic bodies.

The magnetic bodies can be produced, for example, by the following method.

An alkali such as sodium hydroxide or the like in an amount equivalent to the iron component or in a large amount is added to an aqueous ferrous salt solution to prepare an aqueous solution including ferrous hydroxide. Air is blown while maintaining the pH of the prepared aqueous solution at 7 or more, oxidation reaction of ferrous hydroxide is performed while heating the aqueous solution to 70° C. or more, and seed crystals to be the magnetic iron oxide cores are first generated.

Next, an aqueous solution including about 1 equivalent of ferrous sulfate based on the amount of alkali, which has been added previously, is added to the slurry including the seed crystals. The pH of the mixed solution is maintained at 5 to 10, the reaction of ferrous hydroxide is advanced while blowing the air, and magnetic iron oxide is grown on the seed crystals as the cores. At this time, it is possible to control the shape and magnetic properties of the magnetic bodies by selecting any pH, reaction temperature and stirring conditions. As the oxidation reaction proceeds, the pH of the mixture shifts to the acidic side, but the pH of the mixture should not be less than 5. Magnetic bodies can be obtained by filtering, washing and drying the magnetic bodies, which have been thus obtained, according to a conventional method.

In addition, the magnetic bodies may be subjected to known surface treatment as needed.

The dielectric loss tangent of the magnetic toner at 100 kHz is preferably 0.01 or more. The dielectric loss tangent is more preferably from 0.04 to 0.15. The dielectric loss tangent indicates the ratio of the dielectric constant to the dielectric loss ratio, and the larger the value of the dielectric loss tangent, the higher the proportion of the dielectric loss ratio, indicating that charge relaxation after polarization is likely to occur.

In one-component non-contact development, an AC bias is applied to develop a latent image of the photosensitive member between the toner borne on the developer bearing member and the photosensitive member. At that time, it is necessary to control the dielectric loss tangent value of the toner as the sensitivity to the frequency of the AC bias.

Where the dielectric loss tangent is within the above range, the charged state of the toner becomes appropriate even in a low-temperature environment, electrostatic offset is suppressed by not causing excessive charge-up, and a satisfactory image can be obtained.

Where the dielectric loss tangent is 0.01 or more, charge relaxation is likely to occur and it is difficult to retain the

excessive charge. As a result, when the toner is triboelectrically charged in a low-temperature environment, charge-up is unlikely to occur and the electrostatic offset can be suppressed.

The dielectric loss tangent can be controlled by the dispersibility (aggregation) of the magnetic bodies in the toner particle. By dispersing the magnetic bodies in the toner particles without aggregation, dielectric polarization is likely to occur, and the value of the dielectric loss tangent can be reduced. Conversely, the value of the dielectric loss tangent can be increased by causing aggregation and making dielectric polarization less likely to occur. Further, the control can also be performed by the dispersion state of the magnetic bodies among the toner particles.

Here, the frequency to 100 kHz is set as a reference for measuring the dielectric loss tangent because such a frequency is suitable for verifying the dispersion state of the magnetic bodies. Where the frequency is lower than 100 kHz, the dielectric loss tangent becomes small, so it is difficult to understand the change in the dielectric loss tangent of the toner, and where the frequency is higher than 100 kHz, the difference in dielectric loss tangent when the temperature is changed becomes undesirably small.

The binder resin is not particularly limited, and a known resin for toner can be used. Specific examples of the binder resin include amorphous polyester, polyurethane resin, and vinyl resins.

Examples of the monomers that can be used for the production of vinyl resins are listed hereinbelow.

Aliphatic vinyl hydrocarbons: alkenes such as ethylene, propylene, butene, isobutylene, pentene, heptene, diisobutylene, octene, dodecene, octadecene, and other  $\alpha$ -olefins; and alkadienes, such as butadiene, isoprene, 1,4-pentadiene, 1,6-hexadiene and 1,7-octadiene.

Alicyclic vinyl hydrocarbons: mono- or di-cycloalkenes and alkadienes, such as cyclohexene, cyclopentadiene, vinylcyclohexene, and ethylidenebicycloheptene; and terpenes such as pinene, limonene, and indene.

Aromatic vinyl hydrocarbons: styrene and hydrocarbyl (alkyl, cycloalkyl, aralkyl and/or alkenyl) substituents thereof, such as  $\alpha$ -methylstyrene, vinyltoluene, 2,4-dimethylstyrene, ethylstyrene, isopropylstyrene, butylstyrene, phenylstyrene, cyclohexylstyrene, benzylstyrene, crotylbenzene, divinylbenzene, divinyltoluene, divinyxylene, trivinylbenzene; and vinylnaphthalene.

Carboxy group-containing vinyl-based monomers and metal salts thereof unsaturated monocarboxylic acids having from 3 to 30 carbon atoms, unsaturated dicarboxylic acids, anhydrides thereof and monoalkyl (from 1 to 27 carbon atoms) esters thereof. For example, carboxy group-containing vinyl-based monomers such as acrylic acid, methacrylic acid, maleic acid, maleic anhydride, monoalkyl esters of maleic acid, fumaric acid, monoalkyl esters of fumaric acid, crotonic acid, itaconic acid, monoalkyl esters of itaconic acid, glycol monoether itaconate, citraconic acid, citraconic acid monoalkyl esters and cinnamic acid.

Vinyl esters, such as vinyl acetate, vinyl butyrate, vinyl propionate, butyric acid vinyl ester, diallyl phthalate, diallyl adipate, isopropenyl acetate, vinyl methacrylate, methyl 4-vinyl benzoate, cyclohexyl methacrylate, benzyl methacrylate, phenyl acrylate, phenyl methacrylate, vinyl methoxyacetate, vinyl benzoate, ethyl  $\alpha$ -ethoxy acrylate, alkyl acrylates and alkyl methacrylates having an alkyl group (linear or branched) having from 1 to 22 carbon atoms (methyl acrylate, methyl methacrylate, ethyl acrylate, ethyl methacrylate, propyl acrylate, propyl methacrylate, butyl acrylate, butyl methacrylate, 2 ethylhexyl acrylate, 2-ethyl-

hexyl methacrylate, lauryl acrylate, lauryl methacrylate, myristyl acrylate, myristyl methacrylate, cetyl acrylate, cetyl methacrylate, stearyl acrylate, stearyl methacrylate, eicosyl acrylate, eicosyl methacrylate, behenyl acrylate, behenyl methacrylate, and the like), dialkyl fumarates (fumaric acid dialkyl ester, two alkyl groups are linear, branched or alicyclic groups having from 2 to 8 carbon atoms), dialkyl maleates (maleic acid dialkyl ester, two alkyl groups are linear, branched or alicyclic group having from 2 to 8 carbon atoms), polyaryloxyalkanes (diaryloxyethane, triaryloxyethane, tetraaryloxyethane, tetraaryloxypropane, tetraaryloxybutane, and tetramethallyloxyethane), vinyl-based monomers having a polyalkylene glycol chain (polyethylene glycol (molecular weight 300) monoacrylate, polyethylene glycol (molecular weight 300) monomethacrylate, polypropylene glycol (molecular weight 500) monoacrylate, polypropylene glycol (molecular weight 500) monomethacrylate, methyl alcohol ethylene oxide (ethylene oxide is hereinafter abbreviated as EO) 10 mole adduct acrylate, methyl alcohol ethylene oxide 10 mole adduct methacrylate, lauryl alcohol EO 30 mole adduct acrylate, lauryl alcohol EO 30 mole adduct methacrylate), polyacrylates and polymethacrylates (polyacrylates and polymethacrylates of polyhydric alcohols: ethylene glycol diacrylate, ethylene glycol dimethacrylate, propylene glycol diacrylate, propylene glycol dimethacrylate, neopentyl glycol diacrylate, neopentyl glycol dimethacrylate, trimethylolpropane triacrylate, trimethylolpropane trimethacrylate, polyethylene glycol diacrylate, and polyethylene glycol dimethacrylate).

Carboxy group-containing vinyl esters: for example, carboxyalkyl acrylates having an alkyl chain having from 3 to 20 carbon atoms, and carboxyalkyl methacrylates having an alkyl chain having from 3 to 20 carbon atoms.

Among these, styrene, butyl acrylate,  $\beta$ -carboxyethyl acrylate and the like are preferable.

Examples of monomers that can be used for the manufacture of the amorphous polyester include conventionally well-known bivalent, trivalent or higher polyvalent carboxylic acids and dihydric, trihydric or higher polyhydric alcohols. Specific examples of these monomers are listed hereinbelow.

Examples of the divalent carboxylic acids include dibasic acids such as oxalic acid, malonic acid, succinic acid, glutaric acid, adipic acid, pimelic acid, suberic acid, azelaic acid, sebacie acid, 1,9-nonanedicarboxylic acid, 1,10-decanedicarboxylic acid, 1,11-undecanedicarboxylic acid, 1,12-dodecanedicarboxylic acid, 1,13-tridecanedicarboxylic acid, 1,14-tetradecanedicarboxylic acid, 1,16-hexadecanedicarboxylic acid, 1,18-octadecanedicarboxylic acid, phthalic acid, isophthalic acid, terephthalic acid, dodecenyl succinic acid and the like, anhydrides thereof or lower alkyl esters thereof, and aliphatic unsaturated dicarboxylic acids such as maleic acid, fumaric acid, itaconic acid, citraconic acid and the like. Lower alkyl esters of these dicarboxylic acids and acid anhydrides can also be used.

Further, examples of trivalent or higher carboxylic acids include 1,2,4-benzenetricarboxylic acid, 1,2,5-benzenetricarboxylic acid, anhydrides thereof, lower alkyl esters thereof, and the like.

These may be used singly, or two or more thereof may be used in combination.

Examples of dihydric alcohols include alkylene glycols (1,2-ethanediol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-undecanediol, 1,12-dodecanediol, 1,13-tridecanediol, 1,14-tetradecanediol, 1,18-octadecanediol and 1,20-icosanediol); alkylene ether

glycols (polyethylene glycol and polypropylene glycol); alicyclic diols (1,4-cyckhexanedimethanol); bisphenols (bisphenol A); alkylene oxide (ethylene oxide and propylene oxide) adducts of alicyclic diols, and alkylene oxide (ethylene oxide and propylene oxide) adducts of bisphenols (bisphenol A).

The alkyl moieties of the alkylene glycol and the alkylene ether glycol may be linear or branched. In the present invention, an alkylene glycol having a branched structure can also be preferably used.

In addition, aliphatic diols having a double bond can also be used. The following compounds can be mentioned as aliphatic diols having a double bond.

2-Butene-1,4-diol, 3-hexene-1,6-diol and 4-octene-1,8-diol.

Further, examples of the trihydric or higher alcohols include glycerin, trimethylolethane, trimethylolpropane and pentaerythritol.

These may be used singly, or two or more thereof may be used in combination.

For the purpose of adjusting the acid value and the hydroxyl value, a monobasic acid such as acetic acid and benzoic acid, and a monohydric alcohol such as cyclohexanol and benzyl alcohol can also be used, if necessary.

The binder resin preferably includes an amorphous polyester.

Among these, from the viewpoint of paper adhesion, the weight average molecular weight  $M_w$  of the amorphous polyester is preferably 90000 or less.

Further, from the viewpoint of the difference in image density before and after repeated use, the weight average molecular weight is preferably 1500 or more.

A method for synthesizing the amorphous polyester is not particularly limited, and for example, a transesterification method or a direct polycondensation method can be used singly or in combination.

The number average molecular weight  $M_n$  of the amorphous polyester is preferably from 1000 to 50000, and more preferably from 5000 to 40000.

For the amorphous polyester, it is preferable to use succinic acid substituted with an alkenyl group having from 6 to 18 carbon atoms or an anhydride thereof. That is, the amorphous polyester preferably comprises a structure in which succinic acid substituted with an alkenyl group having from 6 to 18 carbon atoms is polycondensed with a polyhydric alcohol. The amorphous polyester more preferably has a structure in which dodeceny succinic acid or an anhydride thereof is polycondensed.

Since the amorphous polyester has a structure derived from alkenyl succinic acid, the crystalline polyester can easily take a crystal structure and the sharp melt property is enhanced.

The amount of the structure in which the succinic acid (preferably dodeceny succinic acid) substituted with an alkenyl group having from 6 to 18 carbon atoms or an anhydride thereof is polycondensed in the amorphous polyester is preferably from 1% by mass to 30% by mass, and more preferably from 5% by mass to 25% by mass.

A resin such as an amorphous polyester, a polyurethane, and a vinyl resin may be used singly or in combination of two or more thereof as the binder resin. From the viewpoint of using crystalline polyester, the binder resin preferably comprises an amorphous polyester, and is more preferably an amorphous polyester. When using two or more types thereof together, the resins may be used in the form of a composite resin in which the resins are chemically bonded together.

From the viewpoint of low-temperature fixability, the glass transition temperature ( $T_g$ ) of the binder resin is preferably from 40.0°C. to 120.0°C.

The magnetic toner particle preferably has a core-shell structure. That is, it is preferable that the magnetic toner particle has a shell layer. Further, it is more preferable that the magnetic toner particle has a core particle including a binder resin, a magnetic body and a crystalline polyester, and a shell layer on the surface of the core particle. The shell layer does not have to cover the entire core particles, and the core particle may be partially exposed.

The amount of the shell layer is preferably from 1 part by mass to 20 parts by mass, and more preferably from 5 parts by mass to 15 parts by mass with respect to 100 parts by mass of the binder resin.

The shell layer preferably comprises an amorphous polyester having an ethylenically unsaturated bond (double bond) (hereinafter, also referred to as "amorphous unsaturated polyester"), and more preferably is made of an amorphous unsaturated polyester. The amorphous unsaturated polyester is not particularly limited as long as it has an ethylenically unsaturated bond in the molecule.

The unsaturated bond equivalent of the amorphous unsaturated polyester is preferably 4000 g/eq or less, more preferably 1500 g/eq or less, and even more preferably 1000 g/eq or less.

The unsaturated bond equivalent refers to the value measured by the following method. The molecular weight per one unsaturated bond is calculated by performing NMR analysis (H analysis) of the resin, identifying the monomer type and composition ratio, and determining the proportion of the monomer having an unsaturated double bond. An amorphous unsaturated polyester is an amorphous polyester having an ethylenically unsaturated bond (for example, a vinyl group or a vinylene group) in the molecule.

Specifically, for example, an amorphous unsaturated polyester may be a condensed polymer of a polyvalent carboxylic acid and a polyhydric alcohol in which a monomer having an ethylenically unsaturated bond (for example, a vinyl group or a vinylene group) serving as an unsaturated polyester component is used as at least one of the polyvalent carboxylic acid and the polyhydric alcohol.

From the viewpoint of stability, the amorphous unsaturated polyester is preferably a condensed polymer of a polyvalent carboxylic acid having an ethylenically unsaturated bond (for example, a vinyl group or a vinylene group) and a polyhydric alcohol. The amorphous unsaturated polyester is more preferably a condensed polymer (that is, a linear polyester) of a divalent carboxylic acid having an ethylenically unsaturated bond (for example, a vinyl group or a vinylene group) and a dihydric alcohol.

When the amorphous unsaturated polyester is a condensed polymer of a polyvalent carboxylic acid having an ethylenically unsaturated bond and a polyhydric alcohol, a polyvalent carboxylic acid having no ethylenically unsaturated bond may be used, if necessary, as a part of the polyvalent carboxylic acid. Specific examples of the polyvalent carboxylic acid having no ethylenically unsaturated bond include the polyvalent carboxylic acid described in the section related to the amorphous polyester.

Examples of the divalent carboxylic acids having an ethylenically unsaturated bond (for example, vinyl group or vinylene group) include fumaric acid, maleic acid, maleic acid anhydride, citraconic acid, mesaconic acid, itaconic acid, glutaconic acid, allylmalonic acid, isopropylidene succinic acid, acetylenedicarboxylic acid, and lower (from 1 to 4 carbon atoms) alkyl esters thereof.

## 15

Examples of trivalent or higher carboxylic acids having an ethylenically unsaturated bond (for example, vinyl group or vinylene group) include aconitic acid, 3-butene-1,2,3-tricarboxylic acid, 4-pentene-1,2,4-tricarboxylic acid, 1-pentene-1,1,4,4-tetracarboxylic acid, and lower (from 1 to 4 carbon atoms) alkyl esters thereof.

These polyvalent carboxylic acids may be used alone or in combination of two or more.

Examples of the dihydric alcohols include bisphenol A, hydrogenated bisphenol A, ethylene oxide or propylene oxide adduct of bisphenol A, 1,4-cyclohexanediol, 1,4-cyclohexanedimethanol, ethylene glycol, diethylene glycol, propylene glycol, dipropylene glycol, 1,3-butanediol, 1,4-butanediol, 1,5-pentanediol, 1,6-hexanediol, 1,9-nonanediol, and neopentyl glycol.

Examples of trihydric or higher alcohols include glycerin, trimethylolethane, trimethylolpropane, and pentaerythritol.

In addition to the polyhydric alcohol, a monovalent acid such as acetic acid and benzoic acid and a monohydric alcohol such as cyclohexanol and benzyl alcohol may be used in combination, if necessary, for the purpose of adjusting the acid value and hydroxy value. These polyhydric alcohols may be used alone or in combination of two or more.

Among the amorphous unsaturated polyesters which are condensed polymers of these polyvalent carboxylic acids and polyhydric alcohols, a condensed polymer of at least one divalent carboxylic acid selected from fumaric acid, maleic acid, and maleic anhydride and a divalent alcohol is preferable.

That is, the unsaturated polyester component of the amorphous unsaturated polyester is preferably a component derived from at least one divalent carboxylic acid selected from fumaric acid, maleic acid, and maleic anhydride.

The proportion of the monomer having an ethylenically unsaturated bond in the total of the polyvalent carboxylic acid and the polyhydric alcohol constituting the amorphous unsaturated polyester is preferably from 5 mol % to 25 mol %, and more preferably from 10 mol % to 22.5 mol %. The proportion of the monomer having an ethylenically unsaturated bond in the total of the polyvalent carboxylic acid and the polyhydric alcohol constituting the amorphous unsaturated polyester is preferably from 1% by mass to 25% by mass, and more preferably from 5% by mass to 20% by mass.

The proportion of the monomer having an ethylenically unsaturated bond (polyvalent carboxylic acid) in the total polyvalent carboxylic acid is preferably from 12.5 mol % to 22.5 mol %, and more preferably from 12.5 mol % to 20 mol %. Further, the proportion of the monomer having an ethylenically unsaturated bond (polyvalent carboxylic acid) to the total polyvalent carboxylic acid is preferably from 10% by mass to 60% by mass, and more preferably from 20% by mass to 50% by mass.

A method for producing the amorphous unsaturated polyester is not particularly limited, and for example, a transesterification method or a direct polycondensation method can be used alone or in combination.

The weight average molecular weight (Mw) of the amorphous unsaturated polyester is, for example, preferably from 30,000 to 300,000, more preferably from 30,000 to 200,000, and even more preferably from 35,000 to 150,000.

The glass transition temperature (Tg) of the amorphous unsaturated polyester is preferably from 50° C. to 80° C., and more preferably from 50° C. to 65° C. The glass transition temperature of the amorphous unsaturated poly-

## 16

ester is determined as the peak temperature of the endothermic peak obtained by differential scanning calorimetry (DSC).

The magnetic toner particle may include a charge control agent. The magnetic toner is preferably a negative-charging toner.

Organometallic complex compounds and chelate compounds are effective as charge control agents for negative charge, and examples thereof include monoazo metal complex compounds; acetylacetone metal complex compounds; metal complex compounds of aromatic hydroxycarboxylic acid or aromatic dicarboxylic acid, and the like.

Specific examples of commercially available products include SPIILON BLACK TRH, T-77, T-95 (Hodogaya Chemical Industry Co., Ltd.), and BONTRON (registered trademark) S-34, S-44, S-54, E-84, E-88, and E-89 (Orient Chemical Industry Co., Ltd.).

The charge control agents can be used singly or in combination of two or more thereof.

From the viewpoint of charge quantity, the amount of the charge control agent is preferably from 0.1 parts by mass to 10.0 parts by mass, and more preferably from 0.1 parts by mass to 5.0 parts by mass with respect to 100 parts by mass of the binder resin.

The glass transition temperature (Tg) of the magnetic toner is preferably from 45.0° C. to 70.0° C., and more preferably from 50.0° C. to 65.0° C.

When the glass transition temperature is in the above range, both storage stability and low-temperature fixability can be achieved at a high level. The glass transition temperature can be controlled by the composition of the binder resin, the type of the crystalline polyester, the molecular weight of the binder resin, and the like.

A method for producing the magnetic toner is not particularly limited, and any of dry production methods (for example, kneading and pulverizing method and the like) and wet production methods (for example, emulsion aggregation method, suspension polymerization method, dissolution and suspension method and the like) may be used.

Among these, it is preferable to use the emulsion aggregation method.

When the emulsion aggregation method is used, it is easy to adjust the variation coefficient of the occupied area ratio of the magnetic body within the above range.

A method for producing toner particles using the emulsion aggregation method will be described with specific examples.

The emulsion aggregation method is roughly divided into the following four steps:

(a) a step of preparing a fine particle-dispersed solution, (b) an aggregation step of forming aggregated particles, (c) a coalescence step of forming toner particles by melting and coalescence, (d) a washing and drying step.

(a) Step of Preparing Fine Particle-Dispersed Solution

A particle-dispersed solution is obtained by dispersing fine particles of each material such as a binder resin, a magnetic body and a crystalline polyester in an aqueous medium.

Examples of the aqueous medium include water such as distilled water, ion exchange water, and the like and alcohols. These may be used singly or in combination of two or more thereof.

An auxiliary agent for dispersing the fine particles in the aqueous medium may be used, surfactants being examples of the auxiliary agent.

Surfactants include anionic surfactants, cationic surfactants, amphoteric surfactants, and nonionic surfactants.

Specific examples include anionic surfactants such as alkylbenzene sulfonates,  $\alpha$ -olefin sulfonates, and phosphoric acid esters; cationic surfactants of amine salt type such as alkylamine salts, amino alcohol fatty acid derivatives, polyamine fatty acid derivatives, and imidazoline, or quaternary ammonium salt type such as alkyl trimethyl ammonium salts, dialkyl dimethyl ammonium salts, alkyl dimethyl benzyl ammonium salts, pyridinium salts, alkyl isoquinolinium salts, and benzethonium chloride; nonionic surfactants such as fatty acid amide derivatives and polyhydric alcohols derivatives; and amphoteric surfactants such as alanine, dodecyldi(aminoethyl) glycine, di(octylaminoethyl) glycine and N-alkyl-N,N-dimethylammonium betaines.

The surfactants may be used singly or in combination of two or more thereof.

A method for preparing the fine particle-dispersed solution can be appropriately selected according to the type of dispersoid.

For example, a method for dispersing the dispersoid by using a general dispersing machine such as a rotary shear type homogenizer, a ball mill a sand mill, a dyno mill or the like having a medium can be mentioned. Moreover, in the case of a dispersoid which dissolves in an organic solvent, the dispersoid may be dispersed in an aqueous medium by using the phase inversion emulsification method. In the phase inversion emulsification method, the material to be dispersed is dissolved in an organic solvent in which the material is soluble, the organic continuous phase (O phase) is neutralized, and then a water medium (W phase) is introduced to perform conversion of resin (so-called phase inversion) from W/O to O/W, induce discontinuous phase formation and disperse in the form of particles in an aqueous medium.

The solvent used in the phase inversion emulsification method is not particularly limited as long as the solvent dissolves the resin, but it is preferable to use a hydrophobic or amphiphilic organic solvent for the purpose of forming droplets.

It is also possible to prepare a fine particle-dispersed solution by carrying out polymerization after forming droplets in an aqueous medium as in emulsion polymerization. Emulsion polymerization is a method for obtaining a fine particle-dispersed solution in which a material is dispersed in an aqueous medium by first mixing a precursor of the material to be dispersed, the aqueous medium, and a polymerization initiator and then stirring or shearing. At this time, an organic solvent or a surfactant may be used as an aid for emulsification. Further, a common apparatus may be used for stirring or shearing, and an example thereof is a common disperser, such as a rotation shear type homogenizer.

When dispersing magnetic bodies, particles with a target diameter of primary particles may be dispersed in an aqueous medium. For the dispersion, for example, a general disperser such as a rotary shear type homogenizer, a ball mill, a sand mill, a dyno mill or the like having media may be used. Since magnetic bodies have a specific gravity higher than that of water and have a high sedimentation rate, it is preferable to immediately proceed to the aggregation step after dispersion.

From the viewpoint of control of aggregation speed and simplicity of coalescence, the number average particle diameter of the dispersoid of the fine particle-dispersed solution is preferably, for example, from 0.01  $\mu\text{m}$  to 1  $\mu\text{m}$ , more preferably from 0.08  $\mu\text{m}$  to 0.8  $\mu\text{m}$ , and even more preferably from 0.1  $\mu\text{m}$  to 0.6  $\mu\text{m}$ .

From the viewpoint of controlling the aggregation speed, the dispersoid in the fine particle-dispersed solution is preferably from 5% by mass to 50% by mass, and more preferably from 10% by mass to 40% by mass based on the total amount of the dispersion.

(b) Aggregation Step

After preparing the fine particle-dispersed solution, one kind of fine particle-dispersed solution or two or more kinds of particle-dispersed solutions are mixed to prepare an 10 aggregated particle-dispersed solution in which aggregated particles in which the fine particles are aggregated are dispersed.

The mixing method is not particularly limited, and the mixing can be performed using a common stirrer.

15 The aggregation is controlled by the temperature, pH, flocculant and the like of the aggregated particle-dispersed solution, and any method may be used.

The temperature at which the aggregated particles are formed is preferably from a glass transition temperature of 20 the binder resin minus 30.0° C. to a glass transition temperature of the binder resin. From an industrial viewpoint, the time is preferably about 1 min to 120 min.

25 The flocculant can be exemplified by inorganic metal salts, metal complexes with a valence of two or more, and the like. When a surfactant is used as an auxiliary agent in the fine particle-dispersed solution, it is also effective to use a surfactant of reverse polarity. In particular, when a metal complex is used as the flocculant, the amount of surfactant used is reduced, and the charging characteristics are 30 improved. Examples of inorganic metal salts include metal salts such as sodium chloride, calcium chloride, calcium nitrate, barium chloride, magnesium chloride, magnesium sulfate, zinc chloride, aluminum chloride, aluminum sulfate and the like, and inorganic metal salt polymers such as 35 polyaluminum chloride, polyaluminum hydroxide, calcium polysulfide and the like.

From the viewpoint of low-temperature fixability and charge retention, the flocculant is preferably a metal salt including at least one metal selected from the group 40 consisting of Mg, Ca, Sr, Al, Fe, and Zn. That is, it is preferable that the magnetic toner particle comprises a polyvalent metal and that the polyvalent metal be at least one metal (more preferably Mg) selected from the group consisting of Mg, Ca, Sr, Al, Fe, and Zn.

45 In the case of the above metal salt, it is easy to contribute to the stability of charging performance before and after durable use.

The total amount of at least one polyvalent metal selected 50 from the group consisting of Mg, Ca, Sr, Al, Fe, and Zn (more preferably, the amount of Mg) in the magnetic toner particle is preferably from 25 ppm to 1000 ppm on a mass basis. Within the above range, sufficient charging performance is maintained even under high temperature and high humidity. More preferably, the total amount is from 30 ppm 55 to 500 ppm.

The timing of mixing of the fine particle-dispersed solution is not particularly limited, and the fine particle-dispersed solution may be further added for aggregation after the aggregated particle-dispersed solution has been formed 60 or in the course of formation.

By controlling the addition timing of the fine particle-dispersed solution, it is possible to control the internal structure of the toner particle.

In order to control the degree of aggregation of the 65 above-mentioned magnetic bodies, for example, a pre-aggregation step of adding the flocculant to the magnetic body-dispersed solution and stirring can be performed

before aggregating each fine particle-dispersed solution. In the pre-aggregation step, for example, it is preferable to add about 0.3 parts by mass to 2.0 parts by mass of the flocculant to 100 parts by mass of the magnetic bodies at about 20° C. to 60° C. and stir for about 5 see to 5 min.

Alternatively, a method is also preferable in which the magnetic body-dispersed solution is added and the aggregation is further performed after the fine particle-dispersed solution other than the magnetic body-dispersed solution is aggregated.

Further, in the aggregation step, a stirring device capable of controlling the stirring speed may be used. The stirring device is not particularly limited, and any general-purpose emulsifying machine and dispersing machine can be used.

For example, a batch-type emulsification machine such as ULTRA TURRAX (manufactured by IKA Corporation), POLYTRON (manufactured by Kinematics Co.), T. K. HOMOMIXER (manufactured by Tokushu Kika Kogyo Co., Ltd.), EBARA MILDNER (manufactured by Ebara Corp.), T. K. HOMOMIC LINE FLOW (manufactured by Tokushu Kika Kogyo Co., Ltd.), CREAMIX (manufactured by M Technique Co., Ltd.), PHILMIX (manufactured by Tokushu Kika Kogyo Co., Ltd.), or both batch-type and continuous-type emulsification machine can be used.

The stirring speed may be appropriately adjusted according to the production scale.

In particular, magnetic bodies having a heavy specific gravity are susceptible to the stirring speed. By adjusting the stirring speed and the stirring time, it is possible to control to the desired particle size. When the stirring speed is high, aggregation is likely to be promoted, aggregation of the magnetic bodies proceeds, and a toner with a low brightness is likely to be finally formed.

Further, when the stirring speed is low, the magnetic bodies tend to settle, the aggregated particle dispersion liquid becomes nonuniform, and a difference is easily caused in the introduction amount of the magnetic bodies between the particles.

Meanwhile, it is also possible to control the aggregation state by adding a surfactant.

It is preferable to terminate the aggregation when the aggregated particles reach the target particle size.

The termination of aggregation can be performed by dilution, temperature control, pH control, addition of a chelating agent, addition of a surfactant, and the like, and the addition of a chelating agent is preferable from the viewpoint of production. Furthermore, it is a more preferable method to terminate the aggregation by addition of a chelating agent and adjustment of pH. When the addition of the chelating agent and the adjustment of the pH are used in combination, it is possible to form a toner particle in which the magnetic bodies are slightly aggregated after the subsequent coalescence step.

Further, from the viewpoint of low-temperature fixability, hot offset resistance, transferability, and charge retention property, it is preferable that the method for producing toner include a metal removal step of adding a chelating compound having a chelating ability with respect to metal ions to a dispersion liquid including toner particles to remove the metal.

The pH can be adjusted by known methods using an aqueous solution of sodium hydroxide or the like. It is preferable to adjust the pH to 7.0 to 11.0, and more preferably to 7.5 to 10.0.

As the chelating agent, a water-soluble chelating agent is preferred. Specific examples of the chelating agent include, for example, hydroxycarboxylic acids such as tartaric acid,

citric acid, gluconic acid and the like, iminodiacid (IDA), nitrilotriacetic acid (NTA), ethylenediaminetetraacetic acid (EDTA) and the like.

The addition amount of the chelating agent is, for example, preferably from 10.0 parts by mass to 100.0 parts by mass, and more preferably from 20.0 parts by mass to 70.0 parts by mass with respect to 100 parts by mass of the magnetic bodies.

(c) Coalescence Step

After forming the aggregated particles, the particles are heated to form toner particles by melting and coalescence. The heating temperature is preferably equal to or higher than the glass transition temperature of the binder resin. For example, 45° C. to 130° C.

Industrially, the time is preferably 1 min to 900 min, and more preferably 5 min to 500 min.

Further, a toner particle having a core/shell structure may be also formed by heating and coalescing the aggregated particles, then mixing the solution in which particles such as resin are dispersed, and further performing the step (b) of forming the aggregated particles and the step (c) of melting and coalescing.

After coalescence, the toner particles can be cooled by known methods. The cooling rate is preferably about 0.1° C./min to 500° C./min.

(d) Washing and Drying Step

Well-known washing method, solid-liquid separation method, and drying method may be used without particular limitation.

However, in the washing step, it is preferable to carry out substitution washing with ion exchange water sufficiently from the viewpoint of charging performance. In the solid-liquid separation step, suction filtration, pressure filtration and the like are preferably performed from the viewpoint of productivity. In the drying step, it is preferable to perform freeze drying, flash jet drying, fluid drying, vibration type fluid drying and the like from the viewpoint of productivity.

The magnetic toner particles may be mixed, if necessary, with an external additive to make the magnetic toner in order to improve the flowability and/or the charging performance of the toner. A known device, for example, a Henschel mixer may be used for mixing of the external additive.

As the external additive, inorganic fine particles having a number average particle diameter of primary particles of from 4 nm to 80 nm are preferable, and inorganic fine particles having a number average particle diameter of primary particles of from 6 nm to 40 nm are more preferable.

The inorganic fine particles can further improve the charging performance and environmental stability of the toner when subjected to a hydrophobization treatment. Examples of treatment agents to be used for the hydrophobization treatment include silicone varnish, various modified silicone varnishes, silicone oils, various modified silicone oils, silane compounds, silane coupling agents, other organic boron compounds, organic titanium compounds and the like. The treatment agents may be used singly or in combination of two or more thereof.

The number average particle diameter of the primary particles of the inorganic fine particles may be calculated using an image of the toner captured by a scanning electron microscope (SEM).

Examples of the inorganic fine particles include silica fine particles, titanium oxide fine particles, alumina fine particles and the like. As the silica fine particles, for example, both dry silica such as silica or fumed silica produced by so-called dry method and generated by vapor phase oxidation

of a silicon halide, and so-called wet silica produced from water glass and the like can be used.

However, dry silica having fewer silanol groups on the surface and inside the silica fine particles and having less production residues such as  $\text{Na}_2\text{O}$  and  $\text{SO}_3^{2-}$  is preferable.

In the production step of dry silica, it is also possible to obtain composite fine particles of silica and other metal oxides, for example, by using other metal halides such as aluminum chloride, titanium chloride and the like together with the silicon halide in the production process, and the concept of dry silica is inclusive of such particles.

The amount of the inorganic fine particles is preferably from 0.1 parts by mass to 3.0 parts by mass with respect to 100 parts by mass of the toner particles. The amount of the inorganic fine particles may be quantitatively determined from a calibration curve prepared from a standard sample using a fluorescent X-ray analyzer.

The magnetic toner may include other additives as long as the effects of the present invention are not adversely affected.

Examples of other additives include lubricant powder such as fluorocarbon resin powder, zinc stearate powder, polyvinylidene fluoride powder and the like; abrasives such as cerium oxide powder, boron carbide powder, strontium titanate powder and the like; anti-caking agents and the like. Other additives can also be used after the surface thereof is hydrophobized.

The volume average particle diameter ( $D_v$ ) of the magnetic toner is preferably from 3.0  $\mu\text{m}$  to 8.0  $\mu\text{m}$ , and more preferably from 5.0  $\mu\text{m}$  to 7.0  $\mu\text{m}$ .

By setting the volume average particle diameter ( $D_v$ ) of the toner within the above range, it is possible to sufficiently satisfy the dot reproducibility while improving toner handleability.

Further, the ratio ( $D_v/D_n$ ) of the volume average particle diameter ( $D_v$ ) to the number average particle diameter ( $D_n$ ) of the magnetic toner is preferably less than 1.25.

The magnetic toner preferably has an average circularity of from 0.970 to 0.985, and more preferably from 0.975 to 0.985.

When the average circularity is in the above range, even in a system with a strong shear force, such as a one-component contact development system, the toner is unlikely to be compacted and the flowability of the toner is easily maintained. As a result, when performing a large number of image outputs, it is possible to further suppress the decrease in fixing separability.

The average degree of circularity may be controlled by a method generally used at the time of toner production. For example, in the emulsion aggregation method, it is preferable to control the duration of the coalescence step and the amount of surfactant added.

Methods for measuring various physical property values according to the present invention are described hereinbelow.

**Method for Calculating Occupied Area Ratio of Magnetic Bodies in Magnetic Toner Particle, Average Value Thereof and Variation Coefficient (CV3) Thereof**

The occupied area ratio of the magnetic bodies in the magnetic toner particle, the average value thereof and the variation coefficient (CV3) thereof are calculated as follows.

First, a transmission electron microscope (TEM) is used to acquire an image of the cross section of the magnetic toner particle. The obtained cross-sectional image is used to obtain a frequency histogram of the occupied area ratio of the magnetic bodies in each divided grid on the basis of a division method.

Then, the variation coefficient of the occupancy area ratio of each obtained division grid is determined and taken as the variation coefficient (CV3) of the occupancy area ratio.

Specifically, first, magnetic toner is compression molded into a tablet. The tablet is obtained by filling a tablet former having a diameter of 8 mm with 100 mg of the magnetic toner, applying a force of 35 kN and allowing to stand for 1 min.

The obtained tablet is cut with an ultrasonic ultramicrotome (Leica Co., Ltd., UC7) to obtain a thin sample having a thickness of 250 nm.

A STEM image of the thin sample obtained is captured using a transmission electron microscope (JEOL Co., JEM 2800).

The probe size used for capturing the STEM image is 1.0 nm, and the image size is 1024×1024 pixels. At this time, by adjusting the Contrast of the bright field image Detector Control panel to 1425, the Brightness to 3750, the Contrast to the Image Control panel to 0.0, the Brightness to 0.5, and the Gamma to 1.00, an image can be captured with only the magnetic body portion being dark. By the setting, a STEM image suitable for image processing can be obtained.

The obtained STEM image is digitized using an image processing apparatus (Nireco, Inc., LUZEX AP).

Specifically, a frequency histogram of the occupied area ratio of the magnetic body in a square grid of 0.8  $\mu\text{m}$  on one side is obtained by the division method. At this time, the grade interval of the histogram is 5%.

Further, the variation coefficient is obtained from the obtained occupied area ratio of each section grid and taken as the variation coefficient CV3 of the occupied area ratio. In addition, the average value of the occupied area ratio is an average of the occupied area ratios of the respective division grids.

**Measurement of Dielectric Loss Tangent of Magnetic Toner**

The dielectric properties of the magnetic toner are measured by the following method.

A total of 1 g of the magnetic toner is weighed, and a load of 20 kPa is applied for 1 min to form a disc-shaped measurement sample having a diameter of 25 mm and a thickness of 1.5±0.5 mm.

The measurement sample is mounted on ARES (manufactured by TA Instruments) equipped with a dielectric measurement jig (electrode) having a diameter of 25 mm. In a state in which a load of 250 g/cm<sup>2</sup> is applied at a measurement temperature of 30° C., the dielectric loss tangent is calculated from the measured value of the complex dielectric constant at 100 kHz and a temperature of 30° C. by using a 4284A Precision LCR meter (manufactured by Hewlett-Packard).

**Method for Measuring Powder Dynamic Viscoelasticity of Magnetic Toner**

The measurement is performed using a dynamic viscoelasticity measuring device DMA 8000 (manufactured by Perkin Elmer Inc.).

Measuring jig: material pocket (P/N: N533-0322)

A total of 80 mg of the magnetic toner is held in the material pocket, and the material pocket is attached to a single cantilever and secured by tightening a screw with a torque wrench.

Measurement is performed using dedicated software "DMA Control Software" (manufactured by Perkin Elmer Inc.). The measurement conditions are as follows.

Oven: Standard Air Oven

Measurement type: temperature scan

DMA condition: single frequency/strain (G)

Frequency: 1 Hz  
 Strain: 0.05 mm  
 Starting temperature: 25° C.  
 End temperature: 180° C.  
 Scanning speed: 20° C./min  
 Deformation mode: single cantilever (B)  
 Cross section: rectangular (R)  
 Specimen size (length): 17.5 mm  
 Specimen size (width): 7.5 mm  
 Specimen size (thickness): 1.5 mm

From the curve of storage elastic modulus  $E'$  obtained by the measurement,  $E'(40)$  and  $E'(85)$  are read, and the value of  $[E'(40)-E'(85)] \times 100/E'(40)$  is calculated.

Methods for measuring various physical property values according to the present invention are described hereinbelow.

**Method for Measuring Volume Average Particle Diameter (D<sub>v</sub>) and Number Average Particle Diameter (D<sub>n</sub>) of Magnetic Toner**

The volume average particle diameter (D<sub>v</sub>) and number average particle diameter (D<sub>n</sub>) of the magnetic toner are calculated in the following manner.

A precision particle diameter distribution measuring apparatus "Coulter Counter Multisizer 3" (registered trademark, manufactured by Beckman Coulter, Inc.) equipped with a 100-μm aperture tube and based on a pore electric resistance method is used as a measuring device. The dedicated software "Beckman Coulter Multisizer 3 Version 3.51" (manufactured by Beckman Coulter, Inc.) provided with the device is used for setting measurement conditions and performing measurement data analysis. The measurement is performed with 25,000 effective measurement channels.

A solution prepared by dissolving special grade sodium chloride in ion exchange water to a concentration of about 1% by mass, for example, "ISOTON II" (manufactured by Beckman Coulter, Inc.), can be used as the electrolytic aqueous solution.

The dedicated software is set up in the following manner before the measurement and analysis.

The total count number in a control mode is set to 50,000 particles on a "CHANGE STANDARD MEASUREMENT METHOD (SOM)" screen in the dedicated software, the number of measurements is set to 1, and a value obtained using "standard particles 10.0 μm" (manufactured by Beckman Coulter, Inc.) is set as a Kd value. The threshold and the noise level are automatically set by pressing the "MEASUREMENT BUTTON OF THE THRESHOLD/NOISE LEVEL". Further, the current is set to 1600 μA, the gain is set to 2, the electrolytic solution is set to ISOTON II, and "FLUSH OF APERTURE TUBE AFTER MEASUREMENT" is checked.

In the "PULSE TO PARTICLE DIAMETER CONVERSION SETTING" screen of the dedicated software, the bin interval is set to a logarithmic particle diameter, the particle diameter bin is set to a 256-particle diameter bin, and a particle diameter range is set from 2 μm to 60 μm.

A specific measurement method is described hereinbelow.

(1) Approximately 200 mL of the electrolytic aqueous solution is placed in a glass 250 mL round-bottom beaker dedicated to Multisizer 3, the beaker is set in a sample stand, and stirring with a stirrer rod is carried out counterclockwise at 24 rev/sec. Dirt and air bubbles in the aperture tube are removed by the "FLUSH OF APERTURE TUBE" function of the dedicated software.

(2) Approximately 30 ml of the electrolytic aqueous solution is placed in a glass 100 mL flat-bottom beaker. Then, about 0.3 mL of a diluted solution obtained by 3-fold mass dilution of "CONTAMINON N" (10% by mass aqueous solution of a neutral detergent for washing precision measuring instruments of pH 7 consisting of a nonionic surfactant, an anionic surfactant, and an organic builder, manufactured by Wako Pure Chemical Industries, Ltd.) with ion exchange water is added.

(3) An ultrasonic disperser "Ultrasonic Dispersion System Tector 150" (manufactured by Nikkaki Bios Co., Ltd.) with an electrical output of 120 W in which two oscillators with an oscillation frequency of 50 kHz are built in with a phase shift of 180 degrees is prepared. About 3.3 L of ion exchange water is placed in the water tank of the ultrasonic disperser, and about 2 mL of CONTAMINON N is added to the water tank.

(4) The beaker of (2) hereinabove is set in the beaker fixing hole of the ultrasonic disperser, and the ultrasonic disperser is actuated. Then, the height position of the beaker is adjusted so that the resonance state of the liquid surface of the electrolytic aqueous solution in the beaker is maximized.

(5) About 10 mg of the magnetic toner is added little by little to the electrolytic aqueous solution and dispersed therein in a state in which the electrolytic aqueous solution in the beaker of (4) hereinabove is irradiated with ultrasonic waves. Then, the ultrasonic dispersion process is further continued for 60 sec. In the ultrasonic dispersion, the water temperature in the water tank is appropriately adjusted to a temperature from 10° C. to 40° C.

(6) The electrolytic aqueous solution of (5) hereinabove in which the toner is dispersed is dropped by using a pipette into the round bottom beaker of (1) hereinabove which has been set in the sample stand, and the measurement concentration is adjusted to be about 5%. Then, measurement is conducted until the number of particles to be measured reaches 50000.

(7) The measurement data are analyzed with the dedicated software provided with the device, and the volume average particle diameter (D<sub>v</sub>) and number average particle diameter (D<sub>n</sub>) are calculated. The "50% D diameter" on the "ANALYSIS/VOLUME STATISTICAL VALUE (ARITHMETIC MEAN)" screen obtained when the graph(% by volume) is set in the dedicated software is taken as the volume average particle diameter (D<sub>v</sub>), and the "ARITHMETIC DIAMETER" on the "ANALYSIS/NUMBER STATISTICAL VALUE (ARITHMETIC MEAN)" screen obtained when the graph(% by number) is set in the dedicated software is taken as the number average particle diameter (D<sub>n</sub>).

**Method for Measuring Average Circularity of Magnetic Toner**

The average circularity of the magnetic toner are measured with a flow-type particle image analyzer "FPTA-3000" (manufactured by Sysmex Corp.) under the measurement and analysis conditions used at the time of calibration operation.

The specific measurement method is described hereinbelow.

First, about 20 mL of ion exchange water from which solid impurities and the like have been removed in advance is placed in a glass container. About 0.2 mL of a diluted solution prepared by diluting "CONTAMINON N" (10% by mass aqueous solution of a neutral detergent for washing

precision measuring instruments of pH 7 consisting of a nonionic surfactant, an anionic surfactant, and an organic builder, manufactured by Wako Pure Chemical Industries, Ltd.) with about three-fold mass of ion exchange water is added as a dispersing agent thereto. Further, about 0.02 g of a measurement sample is added, and dispersion treatment is performed for 2 min using an ultrasonic wave disperser to obtain a dispersion solution for measurement. At that time, the dispersion solution is suitably cooled to a temperature of from 10° C. to 40°C. As the ultrasonic wave disperser, a table-top type ultrasonic cleaner disperser ("VS-150" (manufactured by VELVO-CLEAR Co.)) having an oscillation frequency of 50 kHz and an electric output of 150 W is used, a predetermined amount of ion exchange water is placed into a water tank, and about 2 mL of the CONTAMINON N is added to the water tank.

For measurement, the flow type particle image analyzer equipped with "LUCPLFLN" (magnification 20 $\times$ , numerical aperture 0.40) as the objective lens is used, and a particle sheath "PSE-900A" (manufactured by Sysmex Corporation) is used as a sheath liquid. The dispersion solution prepared according to the procedure is introduced into the flow type particle image analyzer, and 2000 magnetic toner particles are measured in an HPF measurement mode and a total count mode. From the results, the average circularity of the magnetic toner are calculated.

In the measurement, automatic focusing is performed using standard latex particles (for example, "RESEARCH AND TEST PARTICLES Latex Microsphere Suspensions 5100A" manufactured by Duke Scientific Inc. which are diluted with ion exchange water) before the start of the measurement. After that, it is preferable to perform focusing every 2 h from the start of the measurement.

The flow type particle image analyzer used in this case was calibrated by Sysmex Corporation and provided with a calibration certificate issued by Sysmex Corporation.

The measurement is performed under the measurement and analysis conditions at the time of receiving the calibration certification, except that the analysis particle diameter is limited to the circle-equivalent diameter of 1.977  $\mu$ m or more to less than 39.54  $\mu$ m.

#### Method for Measuring Peak Temperature (Or Melting Point) of Maximum Endothermic Peak

The peak temperatures ( $T_m(1)$  and  $T_m(2)$ ) and the endothermic quantity  $H(1)$  of the maximum endothermic peak of are measured under the following conditions using a differential scanning calorimeter (DSC) Q2000 (manufactured by TA Instruments).

Temperature rise rate: 10° C./min

Measurement start temperature: 20° C.

Measurement end temperature: 180° C.

The melting points of indium and zinc are used for temperature correction of the device detection unit, and the melting heat of indium is used for correction of heat quantity.

Specifically, about 5 mg of a sample (magnetic toner) is precisely weighed, placed in an aluminum pan, and measured once. An empty aluminum pan is used as a reference. The peak temperature and the endothermic quantity of the maximum endothermic peak at that time are measured. The endothermic quantity of the endothermic peak is the integral value of the endothermic peak.

The maximum endothermic peak assigned to the crystalline polyester and the maximum endothermic peak assigned to the wax can be distinguished by measuring each material separated by the following method.

#### Method for Separating Each Material from Toner

Each material can be separated from the toner by using the difference in the solubility of each material contained in the toner in a solvent.

5 First separation: the toner is dissolved in methyl ethyl ketone (MEK) at 23° C. to separate soluble components (amorphous resin in binder resin) and insoluble components (crystalline polyester, wax, magnetic bodies, inorganic fine particles, and the like).

10 Second separation: the insoluble components (crystalline polyester, wax, magnetic bodies, inorganic fine particles, and the like) obtained by the first separation are dissolved in MEK at 100° C., and soluble components (crystalline polyester, wax) and insoluble components (magnetic bodies, inorganic fine particles, and the like) are separated.

15 Third separation: the soluble components (crystalline polyester, wax) obtained by the second separation are dissolved in chloroform at 23° C., and the soluble component (crystalline polyester) and the insoluble component (wax) are separated.

20 The peak temperature of the maximum endothermic peak of the separated crystalline polyester and wax is measured and matched with the measurement result of the toner alone.

#### Method for Measuring Glass Transition Temperature (Tg)

25 The glass transition temperature of the magnetic toner or resin can be determined from a reversing heat flow curve at the time of temperature rise obtained by differential scanning calorimetry when measuring the peak temperature of the maximum endothermic peak. The glass transition temperature is a temperature (° C.) at the point where a straight line, which is equidistant in the ordinate direction from the straight line obtained by extending the baseline before and after a specific heat change, and the curve of the stepwise change portion of the glass transition in the reversing heat flow curve cross each other.

#### Method for Measuring Number Average Molecular Weight (Mn), Weight Average Molecular Weight (Mw) and Peak Molecular Weight (Mp) of Resin etc.

30 The number average molecular weight (Mn), weight average molecular weight (Mw) and peak molecular weight (Mp) of the resin and other materials are measured using gel permeation chromatography (GPC) in the following manner.

##### (1) Preparation of Measurement Sample

35 A sample and tetrahydrofuran (THF) are mixed at a concentration of 5.0 mg/mL. The mixture is allowed to stand at room temperature for 5 h to 6 h and then shaken thoroughly, and the sample and THF are mixed well till the sample aggregates are loosened. The components are thereafter allowed to stand for 12 h or more at room temperature. At this time, the time from the start of mixing of the sample and THF to the end of standing is set to be 72 h or more to obtain tetrahydrofuran (THF) soluble matter of the sample.

40 Subsequent filtration through a solvent-resistant membrane filter (pore size: 0.45  $\mu$ m to 0.50  $\mu$ m, Myshory Disc H-25-2 (manufactured by Tosob Corporation)) produces a sample solution.

##### (2) Measurement of Sample

45 Measurement is performed under the following conditions using the obtained sample solution.

Device: high-speed GPC device LC-GPC 150C (manufactured by Waters Co.)

50 Column: 7 series of Shodex GPC KF-801, 802, 803, 804, 805, 806, 807

(manufactured by Showa Denko K.K.)

Mobile phase: THF

Flow rate: 1.0 mL/min

Column temperature: 40° C.

Sample injection volume: 100  $\mu$ L

Detector: RI (refractive index) detector

When measuring the molecular weight of the sample, the molecular weight distribution of the sample is calculated from the relationship between the logarithmic value of the calibration curve prepared using several types of monodispersed polystyrene standard samples and the count number. 5

Samples produced by Pressure Chemical Co. or Tosoh Corporation and having a molecular weight of  $6.0 \times 10^2$ ,  $2.1 \times 10^3$ ,  $4.0 \times 10^3$ ,  $1.75 \times 10^4$ ,  $5.1 \times 10^4$ ,  $1 \times 10^5$ ,  $3.9 \times 10^5$ ,  $8.6 \times 10^5$ ,  $2.0 \times 10^6$ , and  $4.48 \times 10^6$  are used as standard polystyrene samples for preparation of the calibration curve. 10

Method for Measuring Particle Diameter of Dispersion in Fine Particle-Dispersed Solution 15

The particle diameter of the dispersion of each of the fine particle-dispersed solutions such as the resin particle-dispersed solution and the magnetic body-dispersed solution is measured using a laser diffraction/scattering particle size distribution measuring apparatus. Specifically, the measurement is performed in accordance with JIS Z 8825-1 (2001). 20

As a measuring apparatus, a laser diffraction/scattering type particle size distribution measuring apparatus "LA-920" (manufactured by Horiba, Ltd.) is used.

For setting of measurement conditions and analysis of measurement data, dedicated software "HORIBA LA-920 for Windows (registered trademark) WET (LA-920) Ver. 2.02" provided with the LA-920 is used. In addition, ion exchange water from which solid impurities and the like have been removed in advance is used as a measurement solvent. The measurement procedure is as follows. 25

- (1) A batch cell holder is attached to the LA-920.
- (2) A predetermined amount of ion exchange water is poured into a batch cell, and the batch cell is set in the batch cell holder.
- (3) The inside of the batch cell is stirred using a dedicated stirrer tip.
- (4) The "REFRACTIVE INDEX" button on the "DISPLAY CONDITION SETTING" screen is pushed, and the relative refractive index is set to a value corresponding to the particle.
- (5) On the "DISPLAY CONDITION SETTING" screen, the particle diameter standard is set as the volume standard.
- (6) After performing warm-up operation for 1 h or more, adjustment of the optical axis, fine adjustment of the optical axis, and blank measurement are performed.
- (7) A total of 3 mL of the fine particle-dispersed solution is placed in a 100 mL flat bottom beaker made of glass. Then, 57 mL of ion exchange water is added to dilute the fine particle-dispersed solution. Then, about 0.3 mL of a diluted solution prepared by diluting "CONTAMINON N" (10% by mass aqueous solution of a neutral detergent for washing precision measuring instruments of pH 7 consisting of a nonionic surfactant, an anionic surfactant, and an organic builder, manufactured by Wako Pure Chemical Industries, Ltd.) with about three-fold mass of ion exchange water is added as a dispersing agent thereto.
- (8) An ultrasonic disperser "Ultrasonic Dispersion System Tetora 150" (manufactured by Nikkaki Bios Co., Ltd.) with an electrical output of 120 W in which two oscillators with an oscillation frequency of 50 kHz are built in with a phase shift of 180 degrees is prepared. About 3.3 L of ion exchange water is placed in the water tank of the ultrasonic disperser, and about 2 mL of CONTAMINON N is added to the water tank.

(9) The beaker of (7) hereinabove is set in the beaker fixing hole of the ultrasonic disperser, and the ultrasonic disperser is actuated. Then, the height position of the beaker is adjusted so that the resonance state of the liquid surface of the electrolytic aqueous solution in the beaker is maximized.

(10) The ultrasonic dispersion process is further continued for 60 sec. In the ultrasonic dispersion, the water temperature in the water tank is appropriately adjusted to a temperature from 10° C. to 40° C.

(11) The fine particle-dispersed solution prepared in (10) hereinabove is added little by little to the batch cell, while taking care not to cause air bubbles, so that the transmittance of the tungsten lamp is adjusted to 90% to 95%. Then, the particle size distribution is measured. Based on the volume-based particle size distribution data thus obtained, the particle size of the dispersion in the fine particle-dispersed solution is calculated.

Measurement of Total Amount of Polyvalent Metals in Toner Particle

The amount of metals in the toner particles is measured using a multi-element simultaneous ICP emission spectroscopic analyzer Vista-PRO (manufactured by Hitachi High-Tech Science Co., Ltd.).

Sample: 50 mg

Solvent: nitric acid 6 mL

The abovementioned components are weighed and decomposition treatment is performed using a microwave sample pretreatment device ETHOS UP (manufactured by Milestone General K.K.).

Temperature: raised from 20° C. to 230° C. and held at 230° C. for 30 minutes

After passing through filter paper (5C), the decomposition solution is transferred to a 50 mL volumetric flask and the volume is set to 50 mL with ultrapure water. By measuring the aqueous solution in the volumetric flask with the multi-element simultaneous ICP emission spectroscopic analyzer Vista-PRO under the following conditions, the amount of polyvalent metal elements (Mg, Ca, Al, Zn, etc.) and the amount of monovalent metal elements (Na, Li, and K) in the toner particle can be quantified. The amount is quantified by preparing a calibration curve using a standard sample of the element to be quantified and calculating based on the calibration curve.

Conditions: RF power 1.20 kW

Ar gas: plasma flow 15.0 L/min

Auxiliary flow: 1.50 L/min

MFC: 1.50 L/min

Nebuuser flow: 0.90 L/min

Liquid feed pump speed: 15 rpm

Repeated measurement: 3 times

Measurement time: 1.0 s

Measuring Toner to Which Inorganic Fine Particles Including At Least One Metal Selected from Group Consisting of Mg, Ca, Al, and Zn is Externally Added

When measuring the amount of metal in a toner particle of a toner to which inorganic fine particles including at least one metal selected from the group consisting of Mg, Ca, Al, and Zn are externally added, the measurement is performed after the inorganic fine particles are separated from the toner in order to avoid calculating the amount of metal derived from the inorganic fine particles in addition to the metal forming the cross-linking with a polar portion.

The procedure for separating the inorganic fine particles from toner is described hereinbelow.

A total of 6 mL of CONTAMINON N (10% by mass aqueous solution of a neutral detergent for washing preci-

sion measuring instruments of pH 7 consisting of a nonionic surfactant, an anionic surfactant, and an organic builder, manufactured by Wako Pure Chemical Industries, Ltd.) is poured into 100 mL of ion exchange water to prepare a dispersion medium. A total of 5 g of the magnetic toner is added to the dispersion medium and dispersed for 5 minutes with an ultrasonic disperser (AS ONE Corporation, VS-150). After that, the dispersion is set in "KM Shaker" (model: V. SX) manufactured by Iwaki Sangyo Co., Ltd. and shaken for 20 minutes under the condition of 350 cycles per minute.

After that, the toner particles are restrained using a neodymium magnet to remove the supernatant. The precipitated toner particles are collected and dried.

Measurement Method of Oil Absorption by Magnetic Body

The oil absorption by the magnetic body is measured according to the method described in JIS K 5101-1978 (Pigment Test Method: Purified Amani Oil Method).

Specifically, it conforms to the JIS standard.

Measurement Method of Isoelectric Point of Magnetic Particle

The magnetic particles are dissolved or dispersed in ion exchange water at 25°C., and the sample concentration is adjusted to 2.0% by volume. The zeta potential is measured by titrating with 1 mol/L HCl using an ultrasonic zeta potential measuring device DT-1200 (manufactured by Dispersion Technology). The pH when the zeta potential is 0 mV is taken as the isoelectric point.

Measurement of Amount of Magnetic Bodies in Magnetic Toner

The amount of the magnetic bodies in the magnetic toner particle can be measured using a thermal analyzer [TGA7] manufactured by PerkinElmer Corp. The measurement method is as follows. The magnetic toner is heated from room temperature to 900°C. at a heating rate of 25°C./min in a nitrogen atmosphere. The weight loss mass % between 100°C. and 750°C. is the amount of the binder resin, and the residual mass is the amount of the magnetic bodies.

Measurement of Amount of Crystalline Polyester in Binder Resin

First, each material is separated from the toner by using the difference in the solubility of each material contained in the toner in a solvent. The amount of the crystalline polyester is measured based on the following separation.

First separation: the toner is dissolved in methyl ethyl ketone (MEK) at 23°C. to separate soluble components (binder resin) and insoluble components (crystalline polyester, wax, magnetic bodies, inorganic fine particles, and the like).

Second separation: the insoluble components (crystalline polyester, wax, magnetic bodies, inorganic fine particles, and the like) obtained by the first separation are dissolved in MEK at 100°C., and soluble components (crystalline polyester, wax) and insoluble components (magnetic bodies, inorganic fine particles, and the like) are separated.

Third separation: the soluble components (crystalline polyester, wax) obtained by the second separation are dissolved in chloroform at 23°C., and the soluble component (crystalline polyester) and the insoluble component (wax) are separated.

The amount of the crystalline polyester when the total of the first separated binding resin and the third separated crystalline polyester is 100% by mass is calculated.

## EXAMPLES

The present invention will be described hereinbelow in greater detail byway of the following Examples and Comparative Examples, but the present invention is not limited thereto. In the Examples and Comparative Examples, the number of parts and % are all based on mass unless stated otherwise.

25 Production Example of Amorphous Polyester A1  
Terephthalic acid 30.0 parts  
Isophthalic acid 1.2.0 parts  
Dodecetyl succinic acid 0.0 parts  
Trimellitic acid. 4.2 parts  
Bisphenol A ethylene oxide (2 moles) adduct 80.0 parts  
Bisphenol A propylene oxide (2 moles) adduct 74.0 parts  
Dibutyltin oxide 0.1 parts

35 The above materials were placed in a heat-dried two-necked flask, nitrogen gas was introduced into the vessel to maintain the inert atmosphere, and the temperature was raised under stirring. Thereafter, a polycondensation reaction was carried out at 150°C. to 230°C. for about 12 h, and the pressure was gradually reduced at 210°C. to 250°C. to obtain an amorphous polyester A1.

The number average molecular weight (Mn) of the amorphous polyester A1 was 20500, the weight average molecular weight (Mw) was 74100, and the glass transition temperature (Tg) was 58.6°C.

45 Production Examples of Amorphous Polyesters A2 to A5  
Amorphous polyesters A2 to A5 were obtained in the same manner as in Production Example of Amorphous Polyester A1, except that the formulation was changed as shown in Table 1.

TABLE 1

| Amorphous<br>polyester<br>No. | Alcohol<br>component |            | Acid component (Parts) |                     |                  |                 |                     |                 |       | Physical properties |            |  |
|-------------------------------|----------------------|------------|------------------------|---------------------|------------------|-----------------|---------------------|-----------------|-------|---------------------|------------|--|
|                               | (Parts)              |            | Dodecetyl              |                     |                  |                 |                     |                 |       | of resin            |            |  |
|                               | BPA-<br>EO           | BPA-<br>PO | Terephthalic<br>acid   | Isophthalic<br>acid | succinic<br>acid | Sebacic<br>acid | Trimellitic<br>acid | Fumaric<br>acid | Mn    | Mw                  | Tg<br>° C. |  |
| A1                            | 80.0                 | 74.0       | 30.0                   | 12.0                | 37.0             | 0.0             | 4.2                 | 0.0             | 20500 | 74100               | 58.6       |  |
| A2                            | 80.0                 | 74.0       | 40.0                   | 20.0                | 0.0              | 0.0             | 4.2                 | 0.0             | 21000 | 80200               | 58.7       |  |
| A3                            | 80.0                 | 74.0       | 30.0                   | 12.0                | 0.0              | 0.0             | 4.2                 | 30.0            | 15000 | 65000               | 59.0       |  |
| A4                            | 80.0                 | 74.0       | 48.0                   | 0.0                 | 11.5             | 0.0             | 12.5                | 0.0             | 42000 | 128900              | 60.2       |  |
| A5                            | 80.0                 | 74.0       | 30.0                   | 0.0                 | 37.0             | 15.6            | 4.2                 | 0.0             | 2500  | 14600               | 56.9       |  |

In the Table, "Mn" denotes Number average molecular weight, and "Mw" denotes Weight average molecular weight. In the table, the abbreviations are as follows. BPA-EO: bisphenol A ethylene oxide (2 mol) adduct BPA-PO: bisphenol A propylene oxide (2 mol) adduct Production Example of Crystalline Polyester B1 1,10-Decanedicarboxylic acid 79.0 parts 1,6-Hexanediol 56.0 parts Dibutyltin oxide 0.1 parts

The above materials were placed in a heat-dried two-necked flask, nitrogen gas was introduced into the vessel to maintain the inert atmosphere, and the temperature was raised under stirring. Then, stirring was performed at 180° C. for 6 h. Thereafter, the temperature was gradually raised to 230° C. under reduced pressure while the stirring was continued, and the temperature was further maintained for 2 h. A crystalline polyester B1 was synthesized by cooling with air and stopping the reaction once a viscous state was reached. The weight average molecular weight (Mw) of crystalline polyester B1 was 22500, and the melting point was 73.0° C.

#### Production Example of Crystalline Polyesters B2 and B3

Crystalline polyesters B2 and B3 were obtained in the same manner as in the Production Example of Crystalline Polyester B1, except that the formulation was changed as shown in Table 2. These crystalline polyesters had a definite melting point.

TABLE 2

| Crystalline polyester | Alcohol component (parts) |                |                 | Acid component (parts)<br>1,10-Decanedicarboxylic acid | Physical properties of resin |       |           |
|-----------------------|---------------------------|----------------|-----------------|--------------------------------------------------------|------------------------------|-------|-----------|
|                       | 1,6-Hexanediol            | 1,9-Nonanediol | Ethylene glycol |                                                        | Mn                           | Mw    | Tm [° C.] |
| B1                    | 56.0                      | —              |                 | 79.0                                                   | 5700                         | 22500 | 73.0      |
| B2                    |                           | 80.0           | —               | 85.0                                                   | 4900                         | 26700 | 79.0      |
| B3                    | —                         |                | 33.0            | 70.0                                                   | 6300                         | 29100 | 84.0      |

In the Table, "Mn" denotes Number average molecular weight, and "Mw" denotes Weight average molecular weight.

#### Production Example of Resin Particle-Dispersed Solution D-1

A total of 112.5 parts of ethyl acetate, 37.5 parts of the amorphous polyester A1, 0.3 parts of 0.1 mol/L sodium hydroxide, and 0.2 parts of an anionic surfactant (Neogen RK, manufactured by Daiichi Kogyo Seiyaku Co., Ltd.) were placed in a beaker equipped with a stirrer, heating to 60.0° C. was performed, and stirring was continued until complete dissolution to prepare a resin solution D-1.

A total of 112.5 parts of ion exchange water was gradually added while further stirring the resin solution D-1, phase inversion emulsification was carried out, and solvent removal was performed to obtain a resin particle-dispersed solution D-1 (solid fraction concentration: 25.0% by mass).

The volume average particle diameter of the resin particles in the resin particle-dispersed solution D-1 was 0.19  $\mu\text{m}$ .

#### Production Examples of Resin Particle-Dispersed Solutions D-2 to D-8

Resin particle-dispersed solutions D-2 to D-8 were obtained in the same manner as in Production Example of Resin Particle-Dispersed Solution D-1, except that the formulation was changed as shown in Table 3. The formulations and physical properties are shown in Table 3.

TABLE 3

| Resin Particle-dispersed solution | Resin components (parts) |       | Ion exchange water | Particle diameter [ $\mu\text{m}$ ] |
|-----------------------------------|--------------------------|-------|--------------------|-------------------------------------|
|                                   | Type                     | Parts |                    |                                     |
| D-1                               | A1                       | 37.5  | 112.5              | 0.19                                |
| D-2                               | A2                       | 37.5  | 112.5              | 0.18                                |
| D-3                               | A3                       | 37.5  | 112.5              | 0.22                                |
| D-4                               | A4                       | 37.5  | 112.5              | 0.18                                |
| D-5                               | A5                       | 37.5  | 112.5              | 0.22                                |
| D-6                               | B1                       | 37.5  | 112.5              | 0.19                                |
| D-7                               | B2                       | 37.5  | 112.5              | 0.22                                |
| D-8                               | B3                       | 37.5  | 112.5              | 0.19                                |

Production Example of Wax-Dispersed Solution W-1 Paraffin wax (melting point 73° C.) 50.0 parts Anionic surfactant 0.3 parts (Neogen RK, manufactured by Daiichi Kogyo Seiyaku Co., Ltd.)

#### Ion exchange water 150.0 parts

The above components were mixed, heated to 95° C., and dispersed using a homogenizer (ULTRA TURRAX T50, manufactured by IKA Corporation). Thereafter, dispersion was carried out with a Manton-Gaulin high-pressure homogenizer (manufactured by Gaulin Co., Ltd.) to prepare a wax-dispersed solution W-1 (solid fraction concentration:

25% by mass) in which wax particles were dispersed. The volume average particle size of the obtained wax particles was 0.21  $\mu\text{m}$ .

#### Production Example of Wax-Dispersed Solution W-2 Fischer-Tropsch hydrocarbon wax (melting point 105° C.) 50.0 parts

Anionic surfactant 0.3 parts (Neogen RK, manufactured by Daiichi Kogyo Seiyaku Co., Ltd.)

#### Ion exchange water 150.0 parts

The above components were mixed, heated to 95° C., and dispersed using a homogenizer (ULTRA TURRAX T50, manufactured by IKA Corporation). Thereafter, dispersion was carried out with a Manton-Gaulin high-pressure homogenizer (manufactured by Gaulin Co., Ltd.) to prepare a wax-dispersed solution W-2 (solid fraction concentration: 25% by mass) in which wax particles were dispersed. The volume average particle size of the obtained wax particles was 0.22  $\mu\text{m}$ .

#### Production Example of Wax-Dispersed Solution W-3 Fischer-Tropsch hydrocarbon wax (melting point 90° C.) 50.0 parts

Anionic surfactant 0.3 parts (Neogen RK, manufactured by Daiichi Kogyo Seiyaku Co., Ltd.)

#### Ion exchange water 150.0 parts

The above components were mixed, heated to 95° C., and dispersed using a homogenizer (ULTRA TURRAX T50,

manufactured by IKA Corporation). Thereafter, dispersion was carried out with a Manton-Gaulin high-pressure homogenizer (manufactured by Gaulin Co., Ltd.) to prepare a wax-dispersed solution W-3 (solid fraction concentration: 25% by mass) in which wax particles were dispersed. The volume average particle size of the obtained wax particles was 0.23  $\mu\text{m}$ .

#### Production Example of Magnetic Body 1

A total of 55 L of a 4.0 mol/L sodium hydroxide aqueous solution was mixed and stirred with 50 liters of a ferrous sulfate aqueous solution including 2.0 mol/L of  $\text{Fe}^{2+}$  to obtain a ferrous salt aqueous solution including a ferrous hydroxide colloid. The aqueous solution was maintained at 85° C., and an oxidation reaction was carried out for 2 h while blowing in air at 20 L/min to obtain a slurry including core particles.

The obtained slurry was filtered and washed with a filter press, and the core particles were then re-dispersed in water. A total of 0.20% by mass of sodium silicate in terms of silicon per 100 parts of core particles was added to the obtained re-slurry solution, the pH of the slurry solution was adjusted to 6.0, and stirring was performed to obtain magnetic iron oxide particles having a silicon-rich surface.

The obtained slurry solution was filtered with a filter press, washed, and re-slurried with ion exchange water. To this re-slurry solution (solid fraction: 50 parts/L), 500 parts (10% by mass with respect to the magnetic iron oxide) of ion exchange resin SK110 (manufactured by Mitsubishi Chemical Co., Ltd.) was added, and stirring was carried out for 2 h for ion exchange. Thereafter, the ion exchange resin was removed by filtration through a mesh, followed by filtration and washing with a filter press, drying and pulverization to obtain a magnetic body 1 having a number average particle diameter of primary particles of 0.21  $\mu\text{m}$ .

#### Production Example of Magnetic Bodies 2 to 5

Magnetic bodies 2 to 5 were obtained in the same manner as in the Production Example of Magnetic Body 1 except that the oxidation reaction time was adjusted as described in Table 4. Table 4 shows the physical properties of each magnetic body.

#### Production Example of Magnetic Body-Dispersed Solution M-1

Magnetic Body 1 25.0 parts

Ion exchange water 75.0 parts

The above materials were mixed and dispersed for 10 min at 8000 rpm using a homogenizer (ULTRA TURRAX T50, manufactured by IKA Corporation) to obtain a magnetic body-dispersed solution M-1. The volume average particle diameter of the magnetic bodies in the magnetic body-dispersed solution M-1 was 0.21  $\mu\text{m}$ .

#### Production Example of Magnetic Body-Dispersed Solutions M-2 to M-5

Magnetic body-dispersed solutions M-2 to M-5 were produced in the same manner as in the Production Example of Magnetic Body-Dispersed Solution M-1, except that the magnetic body 1 was changed to the magnetic bodies 2 to 5, respectively. The physical properties of each magnetic body are shown in Table 4.

TABLE 25

| Magnetic body-dispersed solution | Physical properties of magnetic body |                             |                              |                      |                                                    |
|----------------------------------|--------------------------------------|-----------------------------|------------------------------|----------------------|----------------------------------------------------|
|                                  | Air blowing amount [L/min]           | Oxidation reaction time [H] | Oil absorption amount [ml/g] | Isoelectric point pH | Number average particle diameter [ $\mu\text{m}$ ] |
| M-1                              | 20                                   | 2                           | 20.0                         | 9.0                  | 0.21                                               |
| M-2                              | 20                                   | 1.5                         | 18.0                         | 7.0                  | 0.20                                               |
| M-3                              | 20                                   | 3                           | 22.0                         | 10.4                 | 0.15                                               |
| M-4                              | 20                                   | 4                           | 25.0                         | 12.0                 | 0.19                                               |
| M-5                              | 20                                   | 1                           | 40.0                         | 6.5                  | 0.22                                               |

#### Production Example of Magnetic Toner Particles 1

##### Aggregation Step

Resin particle-dispersed solution D-1 (solid fraction 25.0% by mass) 104.0 parts

Resin particle-dispersed solution D-6 (solid fraction 25.0% by mass) 56.0 parts

Wax-dispersed solution W-1 (solid fraction 25.0% by mass) 15.0 parts

Magnetic body-dispersed solution M-1 (solid fraction 25.0% by mass) 123.3 parts

The above materials were loaded into a beaker, adjusted to a total number of parts of water of 250 parts, and then adjusted to 30.0° C. Then, the materials were mixed by stirring for 10 minutes at 5000 rpm using a homogenizer (ULTRA TURRAX T50, manufactured by IKA Corporation).

Furthermore, 10.0 parts of 2.0% by mass aqueous solution of magnesium sulfate was gradually added as a flocculant.

The raw material-dispersed solution was transferred to a polymerization kettle equipped with a stirrer and a thermometer, and was heated to 50.0° C. with a mantle heater and stirred to promote the growth of aggregated particles.

After 60 minutes had elapsed, 200.0 parts of a 5.0% by mass aqueous solution of ethylenediaminetetraacetic acid (EDTA) was added to prepare an aggregated particle-dispersed solution 1.

##### Shell Layer Formation Step

Subsequently, the aggregated particle-dispersed solution 1 was adjusted to pH 10.0 by using a 0.1 mol/L sodium hydroxide aqueous solution, and then the aggregated particle-dispersed solution 1 was heated to 85.0° C. and allowed to stand for 180 minutes (maturing time) to coalesce the aggregated particles. Then, 10 parts of the resin particle-dispersed solution D-3 was further added.

After 180 min, a toner particle-dispersed solution 1 in which toner particles were dispersed was obtained. After cooling at a temperature lowering rate of 2.0° C./min, the toner particle-dispersed solution 1 was filtered and washed with ion exchange water, and when the conductivity of the filtrate became 50 mS or less, the cake-shaped toner particles were removed.

Next, the cake-shaped toner particles were loaded in ion exchange water taken in an amount 20 times the mass of the toner particles and stirred by a three-one motor. When the toner particles were sufficiently loosened, re-filtration, washing with flowing water, and solid-liquid separation were performed. The resulting cake-shaped toner particles were pulverized in a sample mill and dried in an oven at 40° C. for 24 h. Further, the obtained powder was pulverized with a sample mill, and additional vacuum drying was performed in an oven at 40° C. for 5 h to obtain magnetic toner particles 1.

## Production Example of Magnetic Toner 1

A total of 0.3 parts of sol-gel silica fine particles having a number average particle diameter of primary particles of 115 nm were added to 100 parts of the magnetic toner particles 1, and mixed using an FM mixer (manufactured by Nippon Coke Kogyo Co., Ltd.). Thereafter, 0.9 parts of hydrophobic silica fine particles that were obtained by treating silica fine particles having a number average particle diameter of primary particles of 12 nm with hexamethyldisilazane and then treating with silicone oil and that had a BET specific surface area value of 120 m<sup>2</sup>/g after the treatment were added, and mixing was similarly performed

using the FM mixer (manufactured by Japan Coke Industry Co., Ltd.) to obtain a magnetic toner 1.

The following results relating to the obtained magnetic toner 1 are shown in Table 6.

## Production Example of Magnetic Toner Particles 2 to 29

Magnetic toner particles 2 to 29 were obtained in the same manner as in the Production Example of Magnetic Toner Particles 1, except that the conditions of the aggregation step and the shell layer formation step were changed to the conditions shown in Tables 5 and 6.

For the magnetic toners 19 to 22, a 5.0% by mass of aqueous solution of citric acid was used as the chelating agent.

TABLE 5

TABLE 5-continued

In the Tables 5 and 6, “DS” indicates Dispersed solution “Floc.” indicates Flocculant, Temp. indicates Temperature, “AC” indicates “Aqueous solution of chelating agent”, “AT” indicates “Aggregation time”, and “MT” indicates “Maturing time”.

TABLE 6

TABLE 6-continued

| Toner | Aggregation step |        |            |               |              |      |                 | Shell layer formation step |        |        |            |              |     |
|-------|------------------|--------|------------|---------------|--------------|------|-----------------|----------------------------|--------|--------|------------|--------------|-----|
|       | No. particle     | DS No. | DS [Parts] | Floc. [Parts] | Temp. [° C.] | pH   | Chelating agent | AC [Parts]                 | AT min | DS No. | DS [Parts] | Temp. [° C.] | pH  |
| 29    | D-5              | 160.1  | 10         | 50            | 10.0         | EDTA | 200             | 60                         | —      | —      | 85         | 8.0          | 180 |
|       | D-7              | 14.9   |            |               |              |      |                 |                            |        |        |            |              |     |
|       | W-1              | 15.0   |            |               |              |      |                 |                            |        |        |            |              |     |
|       | M-1              | 155.5  |            |               |              |      |                 |                            |        |        |            |              |     |

## Example 1

## Image Forming Apparatus

The evaluation apparatus is a commercially available magnetic one-component printer HP LaserJet Enterprise M609dn (manufactured by Hewlett-Packard Co., Ltd., process speed 420 mm/s). Using this evaluation apparatus, the following evaluation using toner 1 was carried out.

## Evaluation of Image Density Under Low-Temperature and Low-Humidity Environment

A total of 100 g of the magnetic toner 1 was filled in the apparatus modified as described above, and a repeated use test was performed under a low temperature and low humidity environment (15.0° C./10.0% RH).

As an output image for the test, 4000 prints of horizontal line images with a print percentage of 1% were printed by intermittent sheet passing.

In addition, business 4200 (manufactured by Xerox Co., Ltd.) with a basis weight of 75 g/m<sup>2</sup> was used for the evaluation paper to be used for a test.

A solid black image portion was formed, and the density of the solid black image was measured with a Macbeth reflection densitometer (manufactured by Macbeth Co.).

The criteria for determining the reflection density of the solid black image before the repeated use are as follows.

## Evaluation Criteria

- A: 1.45 or more
- B: 1.40 or more and less than 1.45
- C: 1.35 or more and less than 1.40
- D: less than 1.35

The criteria for determining the image density change (uniformity) after the repeated use are as follows.

The smaller the difference between the reflection density of the solid black image before the repeated use and the reflection density of the solid black image output after printing 4000 prints in the repeated use test, the better.

## Evaluation Criteria

- A: difference in density is less than 0.10
- B: difference in density is 0.10 or more and less than 0.15
- C: difference in density is 0.15 or more and less than 0.20
- D: difference in density is 0.20 or more

## Evaluation of Electrostatic Offset Under Low-Temperature and Low-Humidity Environment

In the evaluation, the temperature of the fixing unit of the image forming apparatus was set at 180° C., a 3 cm square isolated dot image (set to an image density of from 0.75 to 0.80) was outputted to Fox RIVER BOND paper (90 g/m<sup>2</sup>) that was allowed to stand for 24 h under the low-temperature and low-humidity environment (15.0° C./10.0% RH), and

then the level of electrostatic offset generated in a solid white area downstream of the dot image was visually determined.

## Evaluation Criteria

- A: cannot be confirmed visually
- B: very slight level can be confirmed
- C: an offset part can be visually confirmed, but there is also a part that is not offset
- D: 3 cm square can be clearly identified

## Evaluation of Fixing Separability

The evaluation environment was under a normal temperature and normal humidity environment (25.0° C./50% RH), by using the abovementioned image forming apparatus and business 4200 (manufactured by Xerox Co.) having a basis weight of 75 g/m<sup>2</sup> as evaluation paper.

Then, a solid black image having a length of 5.0 cm and a width of 20.0 cm was formed using the filled toner on the recording medium so as to have a toner laid-on level of 0.90 mg/cm<sup>2</sup>. At this time, image formation was performed while changing the range of the margin portion at the upper end in the sheet passing direction.

The unfixed image was fixed at a set temperature of 160° C. The minimum margin at which the paper did not wrap around the fixing roller was evaluated according to the following criteria.

## Evaluation Criteria

- A: no wrapping
- B: the margin from the upper end is 1 mm or more and less than 4 mm
- C: the margin from the upper end is 4 mm or more and less than 7 mm
- D: the margin from the upper end is 7 mm or more

## Evaluation of Heat-Resistant Storability

A total of 10 g of toner to be evaluated was put in a 100 ml resin cup and allowed to stand in an environment of 53° C. for 3 days, and then the state of the powder was visually evaluated.

## Evaluation Criteria

- A: no aggregation was confirmed at all, and the state was substantially the same as the initial state.
- B: the powder appeared aggregated, but could be easily loosened with a finger.
- C: the powder aggregated, but could be loosened with a finger.
- D: the powder solidified.

## Evaluation of Low-Temperature Fixability

The evaluation was performed under a normal temperature and normal humidity environment (25.0° C./50% RH), by using the abovementioned image forming apparatus and

business 4200 (manufactured by Xerox Co.) having a basis weight of 75 g/m<sup>2</sup> as evaluation paper.

#### Speckling

The evaluation image was a solid black image, and the set temperature of the fixing unit of the image forming apparatus was adjusted to 140° C. During the evaluation, the fixing device was removed, and the following evaluation was carried out with the fixing device sufficiently cooled using a tan or the like. By sufficiently cooling the fixing device after the evaluation, the temperature of the fixing nip portion which has been raised after the image output is cooled, so that the fixability of the toner can be strictly evaluated with satisfactory reproducibility.

The toner 1 was used to output a solid black image on the above-mentioned paper in the state where the fixing device was sufficiently cooled. At this time, the toner laid-on level on the paper was adjusted to be 0.90 mg/cm<sup>2</sup>. In the evaluation results of toner 1, a satisfactory solid black image with no speckling was obtained. The determination criteria for the speckling are described below.

The level of speckling was visually evaluated for the solid black image outputted according to the above-mentioned procedure. The determination criteria are as follows.

#### Evaluation Criteria

- A: speckling is completely absent
- B: some speckling is seen upon close examination
- C: speckling is seen, but is not conspicuous
- D: speckling is conspicuous

#### Evaluation of Paper Adhesion

The evaluation image was a halftone image, and the image was outputted by decreasing the set temperature of the fixing unit of the image forming apparatus from 200° C. by 5° C. Then, the fixed image was rubbed ten times with silbon paper under a load of 55 g/cm<sup>2</sup>, and the temperature at which the density reduction rate of the fixed image after rubbing exceeded 10% was taken as the lower limit fixing temperature.

The evaluation was performed according to the following determination criteria. The lower the fixing lower limit temperature, the better the low-temperature fixability.

#### Evaluation Criteria

- A: less than 150° C.
- B: 15° C. or more and less than 160° C.
- C: 160° C. or more and less than 175° C.
- D: 175° C. or more

TABLE 7

| Toner<br>No. | Dn<br>(μm) | CV3  | 10 <sup>9</sup><br>(Pa) | E'(85) ×<br>100/E'(40) | [E'(40) - E'<br>(85)] ×<br>Tm(2) -<br>Tm(1) |       |       | H(1) | Amount<br>of CPES<br>mass % | Amount<br>of MB<br>mass % | DL    | TC   | A |
|--------------|------------|------|-------------------------|------------------------|---------------------------------------------|-------|-------|------|-----------------------------|---------------------------|-------|------|---|
|              |            |      |                         |                        | Tm(2)                                       | Tm(1) | Tm(2) |      |                             |                           |       |      |   |
| 1            | 6.59       | 56.0 | 0.5                     | 75                     | 15.0                                        | 70.0  | 15.0  | 35.0 | 40.0                        | 0.10                      | 0.981 | 101  |   |
| 2            | 6.57       | 52.0 | 0.4                     | 78                     | 15.0                                        | 70.0  | 20.0  | 40.0 | 40.0                        | 0.08                      | 0.982 | 102  |   |
| 3            | 6.86       | 48.0 | 0.3                     | 82                     | 15.0                                        | 70.0  | 25.0  | 50.0 | 40.0                        | 0.06                      | 0.984 | 99   |   |
| 4            | 6.85       | 56.0 | 1.2                     | 72                     | 15.0                                        | 70.0  | 15.0  | 35.0 | 40.0                        | 0.10                      | 0.981 | 101  |   |
| 5            | 6.03       | 45.0 | 0.5                     | 71                     | 15.0                                        | 70.0  | 15.0  | 35.0 | 40.0                        | 0.09                      | 0.979 | 100  |   |
| 6            | 6.79       | 42.0 | 0.7                     | 73                     | 15.0                                        | 70.0  | 12.0  | 35.0 | 40.0                        | 0.05                      | 0.981 | 99   |   |
| 7            | 6.71       | 56.0 | 0.1                     | 73                     | 15.0                                        | 70.0  | 15.0  | 35.0 | 40.0                        | 0.08                      | 0.954 | 99   |   |
| 8            | 6.35       | 75.0 | 0.2                     | 73                     | 15.0                                        | 70.0  | 16.0  | 35.0 | 40.0                        | 0.08                      | 0.975 | 100  |   |
| 9            | 6.88       | 42.0 | 0.5                     | 75                     | 45.0                                        | 100.0 | 15.0  | 35.0 | 40.0                        | 0.07                      | 0.975 | 98   |   |
| 10           | 6.41       | 38.0 | 0.5                     | 78                     | 50.0                                        | 105.0 | 15.0  | 35.0 | 40.0                        | 0.05                      | 0.975 | 103  |   |
| 11           | 6.11       | 72.0 | 0.5                     | 75                     | 15.0                                        | 70.0  | 15.0  | 35.0 | 40.0                        | 0.05                      | 0.975 | 98   |   |
| 12           | 6.76       | 75.0 | 0.2                     | 73                     | 15.0                                        | 70.0  | 15.0  | 35.0 | 12.0                        | 0.10                      | 0.981 | 96   |   |
| 13           | 6.54       | 42.0 | 0.9                     | 78                     | 15.0                                        | 70.0  | 15.0  | 35.0 | 48.0                        | 0.20                      | 0.972 | 95   |   |
| 14           | 6.41       | 78.0 | 1.0                     | 78                     | 15.0                                        | 70.0  | 15.0  | 35.0 | 40.0                        | 0.02                      | 0.982 | 98   |   |
| 15           | 6.11       | 60.0 | 0.7                     | 78                     | 15.0                                        | 70.0  | 15.0  | 35.0 | 40.0                        | 0.02                      | 0.983 | 20   |   |
| 16           | 6.49       | 63.0 | 0.9                     | 78                     | 15.0                                        | 70.0  | 15.0  | 35.0 | 40.0                        | 0.005                     | 0.981 | 1050 |   |
| 17           | 6.71       | 42.0 | 1.9                     | 73                     | 20.0                                        | 70.0  | 15.0  | 35.0 | 40.0                        | 0.09                      | 0.983 | 99   |   |
| 18           | 6.14       | 78.0 | 1.8                     | 72                     | 25.0                                        | 70.0  | 15.0  | 35.0 | 40.0                        | 0.08                      | 0.981 | 100  |   |
| 19           | 6.08       | 30.0 | 0.1                     | 72                     | 15.0                                        | 70.0  | 15.0  | 35.0 | 40.0                        | 0.09                      | 0.984 | 30   |   |
| 20           | 6.59       | 85.0 | 3.9                     | 72                     | 15.0                                        | 70.0  | 15.0  | 35.0 | 40.0                        | 0.08                      | 0.981 | 103  |   |
| 21           | 7.06       | 30.0 | 0.2                     | 80                     | 15.0                                        | 70.0  | 15.0  | 35.0 | 40.0                        | 0.08                      | 0.983 | 50   |   |
| 22           | 6.91       | 85.0 | 4.0                     | 80                     | 15.0                                        | 70.0  | 15.0  | 35.0 | 40.0                        | 0.09                      | 0.984 | 400  |   |
| 23           | 6.15       | 74.8 | 2.3                     | 68                     | 50.0                                        | 105.0 | 15.0  | 14.3 | 55.0                        | 0.15                      | 0.975 | 96   |   |
| 24           | 6.82       | 64.7 | 2.1                     | 68                     | 50.0                                        | 105.0 | 15.0  | 18.2 | 55.0                        | 0.15                      | 0.971 | 95   |   |
| 25           | 6.89       | 43.5 | 4.0                     | 43                     | 50.0                                        | 105.0 | 10.0  | 10.0 | 55.0                        | 0.09                      | 0.972 | 98   |   |
| 26           | 6.85       | 25.4 | 4.0                     | 42                     | 50.0                                        | 105.0 | 8.5   | 8.5  | 55.0                        | 0.11                      | 0.982 | 95   |   |
| 27           | 6.50       | 84.3 | 4.0                     | 42                     | 50.0                                        | 105.0 | 8.5   | 8.5  | 55.0                        | 0.11                      | 0.982 | 98   |   |
| 28           | 6.89       | 62.7 | 6.2                     | 31                     | 50.0                                        | 105.0 | 8.5   | 8.5  | 55.0                        | 0.14                      | 0.971 | 97   |   |
| 29           | 6.29       | 62.7 | 3.2                     | 29                     | 50.0                                        | 105.0 | 8.5   | 8.5  | 55.0                        | 0.14                      | 0.983 | 98   |   |

In the table, "CPES" indicates "crystalline polyester", "MB" indicates "magnetic bodies", "DL" indicates "Dielectric loss tangent of toner", "TC" indicates "Toner average circularity". The amount of crystalline polyester is based on the total content of the binder resin and crystalline polyester. The amount of magnetic bodies is the amount in the magnetic toner. "A" indicates the total amount (ppm) of the polyvalent metal (Mg, Ca, Sr, Al, Fe, and Zn).

Examples 2 to 18 and Comparative Examples 1 to 11

The same evaluation as in Example 1 was carried out using magnetic toners 2 to 29. The results are shown in Table 8.

TABLE 8

| Example No. | Toner No. | Image density under low-temperature and low-humidity environment |               |      | Electrostatic offset Rank | Fixing separability Rank | Heat-resistant storage ability Rank | Low-temperature fixability |                   |
|-------------|-----------|------------------------------------------------------------------|---------------|------|---------------------------|--------------------------|-------------------------------------|----------------------------|-------------------|
|             |           | Rank                                                             | Image density | Rank |                           |                          |                                     | Rank                       | Adhesion to paper |
| 1           | 1         | A                                                                | 1.47          | A    | 0.05                      | A                        | A                                   | A                          | A                 |
| 2           | 2         | B                                                                | 1.41          | A    | 0.06                      | A                        | A                                   | A                          | A                 |
| 3           | 3         | A                                                                | 1.48          | A    | 0.07                      | A                        | A                                   | A                          | A                 |
| 4           | 4         | B                                                                | 1.41          | A    | 0.08                      | A                        | A                                   | C                          | A                 |
| 5           | 5         | A                                                                | 1.46          | C    | 0.17                      | B                        | C                                   | B                          | A                 |
| 6           | 6         | C                                                                | 1.37          | A    | 0.08                      | B                        | C                                   | A                          | C                 |
| 7           | 7         | C                                                                | 1.37          | C    | 0.16                      | C                        | A                                   | A                          | A                 |
| 8           | 8         | B                                                                | 1.41          | B    | 0.12                      | A                        | B                                   | A                          | A                 |
| 9           | 9         | A                                                                | 1.47          | B    | 0.11                      | A                        | A                                   | A                          | B                 |
| 10          | 10        | B                                                                | 1.41          | A    | 0.08                      | C                        | C                                   | A                          | C                 |
| 11          | 11        | C                                                                | 1.36          | B    | 0.13                      | A                        | A                                   | C                          | A                 |
| 12          | 12        | C                                                                | 1.36          | A    | 0.09                      | A                        | A                                   | B                          | C                 |
| 13          | 13        | A                                                                | 1.47          | B    | 0.14                      | A                        | B                                   | A                          | A                 |
| 14          | 14        | C                                                                | 1.36          | A    | 0.08                      | A                        | C                                   | A                          | B                 |
| 15          | 15        | B                                                                | 1.42          | B    | 0.14                      | A                        | A                                   | A                          | A                 |
| 16          | 16        | C                                                                | 1.37          | A    | 0.09                      | C                        | A                                   | A                          | B                 |
| 17          | 17        | A                                                                | 1.48          | A    | 0.08                      | A                        | A                                   | B                          | A                 |
| 18          | 18        | A                                                                | 1.47          | A    | 0.06                      | A                        | A                                   | B                          | A                 |
| C.E. 1      | 19        | D                                                                | 1.32          | A    | 0.09                      | C                        | C                                   | A                          | B                 |
| C.E. 2      | 20        | D                                                                | 1.33          | D    | 0.21                      | D                        | A                                   | A                          | C                 |
| C.E. 3      | 21        | D                                                                | 1.25          | A    | 0.08                      | C                        | D                                   | A                          | B                 |
| C.E. 4      | 22        | C                                                                | 1.37          | D    | 0.22                      | D                        | A                                   | A                          | C                 |
| C.E. 5      | 23        | C                                                                | 1.36          | C    | 0.16                      | C                        | A                                   | B                          | A                 |
| C.E. 6      | 24        | A                                                                | 1.46          | B    | 0.14                      | A                        | A                                   | D                          | D                 |
| C.E. 7      | 25        | D                                                                | 1.27          | A    | 0.06                      | D                        | A                                   | A                          | C                 |
| C.E. 8      | 26        | A                                                                | 1.46          | A    | 0.09                      | C                        | D                                   | A                          | C                 |
| C.E. 9      | 27        | D                                                                | 1.25          | C    | 0.16                      | C                        | C                                   | A                          | C                 |
| C.E. 10     | 28        | A                                                                | 1.46          | A    | 0.08                      | D                        | A                                   | A                          | D                 |
| C.E. 11     | 29        | A                                                                | 1.46          | D    | 0.23                      | C                        | D                                   | D                          | C                 |

In the Table, "C.E." indicates "Comparative Example".

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2020-023197, filed Feb. 14, 2020, which is hereby incorporated by reference herein in its entirety.

What is claimed is:

1. A magnetic toner, comprising:  
a magnetic toner particle comprising a binder resin, a magnetic body and a crystalline polyester;  
the binder resin comprising an amorphous polyester having a structure in which isophthalic acid, terephthalic acid, dodecetyl succinic acid, and trimellitic acid is polycondensed with a polyhydric alcohol;

60 which satisfies  $5.0 \leq Tm(2) - Tm(1) \leq 35.0$

$55.0 \leq Tm(2) \leq 100$  and

$H(1) \geq 10.0$

65 when  $Tm(1)^\circ C$  is the peak temperature of the maximum endothermic peak of the crystalline polyester at the time of the first temperature rise in differential scanning calorimetry

the crystalline polyester comprising a monomer unit derived from 1,6-hexanediol, 1,9-nanandiol, or ethylene glycol, and a monomer unit derived from 1,10-decanedicarboxylic acid; and

5 the crystalline polyester being contained in an amount of 30.0% by mass or more based on the total amount of the binder resin and the crystalline polyester, wherein the magnetic toner has been produced by an emulsion aggregation method,

10 the magnetic body has an oil absorption amount of 15.0 to 25.0 ml/100 g and an isoelectric point of pH 8.5 to 10.5,

a variation coefficient CV3 of an occupied area ratio of the magnetic body is 40.0 to 80.0% when a cross-section of the magnetic toner particle observed using a transmis-

**45**

of the magnetic toner,  $H(1)$  J/g is the endothermic quantity of the maximum endothermic peak, and  $T_m(2^\circ)$  C. is the peak temperature of the maximum endothermic peak assigned to wax.

3. The magnetic toner according to claim 1, wherein the 5 magnetic toner has a dielectric loss tangent at 100 kHz of 0.01 or more.

4. The magnetic toner according to claim 1, wherein the magnetic toner particle has a shell layer comprising an amorphous polyester having an ethylenically unsaturated 10 bond.

5. The magnetic toner according to claim 1, wherein the amount of the magnetic bodies in the magnetic toner is 10.0 to 50.0% by mass.

6. The magnetic toner according to claim 1, wherein the 15 magnetic toner has an average circularity of 0.970 to 0.985.

7. The magnetic toner according to claim 1, wherein the magnetic toner particle further comprises at least one polyvalent metal selected from the group consisting of Mg, Ca, 20 Sr, Al, Fe and Zn, and

the total amount of the polyvalent metal in the magnetic toner particle is 25 to 1000 ppm on a mass basis.

**46**

\* \* \* \* \*